



US009951290B2

(12) **United States Patent**  
**Gao et al.**

(10) **Patent No.:** **US 9,951,290 B2**  
(b4) **Date of Patent:** **Apr. 24, 2018**

(54) **LUBRICANT COMPOSITIONS**

(71) Applicant: **ExxonMobil Research and Engineering Company**, Annandale, NJ (US)

(72) Inventors: **Jason Z. Gao**, Rose Valley, PA (US); **Samuel C. Bainbridge**, Philadelphia, PA (US); **Luca Salvi**, Philadelphia, PA (US)

(73) Assignee: **EXXONMOBIL RESEARCH AND ENGINEERING COMPANY**, Annandale, NJ (US)

(\*) Notice: Subject to any disclaimer, the term of this patent is extended or adjusted under 35 U.S.C. 154(b) by 0 days.

(21) Appl. No.: **15/086,892**

(22) Filed: **Mar. 31, 2016**

(65) **Prior Publication Data**

US 2017/0283731 A1 Oct. 5, 2017

(51) **Int. Cl.**

**C10M 139/00** (2006.01)  
**C10M 137/10** (2006.01)

(Continued)

(52) **U.S. Cl.**

CPC ..... **C10M 141/10** (2013.01); **C10M 139/00** (2013.01); **C10M 141/12** (2013.01); **C10M 2207/28** (2013.01); **C10M 2207/2805** (2013.01); **C10M 2215/223** (2013.01); **C10M 2219/066** (2013.01); **C10M 2219/106** (2013.01); **C10M 2223/045** (2013.01); **C10M 2227/061** (2013.01); **C10N 2210/06** (2013.01); **C10N 2230/06** (2013.01); **C10N 2230/12** (2013.01);

(Continued)

(58) **Field of Classification Search**

CPC ..... C10M 2227/061; C10M 2223/045  
USPC ..... 508/198, 369  
See application file for complete search history.

(56) **References Cited**

## U.S. PATENT DOCUMENTS

|             |         |         |
|-------------|---------|---------|
| 1,815,022 A | 7/1931  | Davis   |
| 2,015,748 A | 10/1935 | Frolich |

(Continued)

## FOREIGN PATENT DOCUMENTS

|               |        |
|---------------|--------|
| CA 1094044 A  | 1/1981 |
| EP 0316610 A1 | 5/1989 |

(Continued)

## OTHER PUBLICATIONS

The International Search Report and Written Opinion of PCT/US2017/020566 dated Sep. 4, 2017.

(Continued)

*Primary Examiner* — Vishal Vasisth

(74) *Attorney, Agent, or Firm* — Robert A. Migliorini

(57) **ABSTRACT**

A method for improving corrosion protection and friction coefficient in an engine or other mechanical component lubricated with a lubricating oil by using as the lubricating oil a formulated oil. The formulated oil has a composition comprising a lubricating oil base stock as a major component, and a mixture of (i) at least one organic molybdenum compound, and (ii) at least one borated ester, as a minor component. Corrosion protection and friction coefficient are improved as compared to corrosion protection and friction coefficient achieved using a lubricating oil containing a minor component other than the mixture of (i) at least one organic molybdenum compound, and (ii) at least one borated ester.

**2 Claims, 9 Drawing Sheets**

|                                                  | 12-89567              | 13-83873  | 13-84096  | 14-38821  | 15-83796  |
|--------------------------------------------------|-----------------------|-----------|-----------|-----------|-----------|
|                                                  | Comparative Example 1 | Example 1 | Example 2 | Example 3 | Example 4 |
| Monocester                                       | 20                    | 20        | 20        | 20        | 20        |
| Other Synthetic Base Oil and Viscosity Modifier  | 68.5                  | 68.18     | 67.692    | 68.674    | 67.76     |
| Molyvan I. (Moly/Sulfur Ratio: 1/1.4, w/w)       | 1.7                   | 1.22      | 1.708     |           |           |
| Sakura-Lube 300 (Moly/Sulfur Ratio: 1/1.07, w/w) |                       |           |           | 1.526     | 2.44      |
| Mixture of 2ndary ZDDPs                          | 1.2                   | 1.2       | 1.2       | 1.2       | 1.2       |
| Other Additives                                  | 8.6                   | 8.6       | 8.6       | 8.6       | 8.6       |
| VANLUBE 289                                      |                       | 0.8       | 0.8       |           |           |
| PX-3871                                          |                       |           |           |           |           |
|                                                  | 100                   | 100       | 100       | 100       | 100       |
| ASTM D130, 150C, 3 hrs                           | 48                    | 2C        | 38        | 1A        | 1A        |
| ASTM D5185 BORON, PPM                            | 250                   | 330       | 320       | 240       | 240       |
| ASTM D5185 CALCIUM, PPM                          | 1630                  | 1680      | 1650      | 1670      | 1630      |
| ASTM D5185 MAGNESIUM, PPM                        | 7.8                   | 3.4       | 3.3       | 8         | 3.4       |
| ASTM D5185 MOLYBDENUM, PPM                       | 1490                  | 1000      | 1400      | 1400      | 1200      |
| ASTM D5185 PHOSPHORUS, PPM                       | 2230                  | 1890      | 2140      | 1630      | 2010      |
| ASTM D5185 ZINC, PPM                             | 1350                  | 1290      | 1300      | 1320      | 1340      |
| MTM Friction Coefficient (140C)                  | 0.058                 | 0.03      | 0.029     | 0.049     | 0.046     |

- (51) **Int. Cl.**
- C10M 141/10* (2006.01) 4,234,435 A 11/1980 Meinhardt et al.  
*C10M 141/12* (2006.01) 4,239,930 A 12/1980 Allphin et al.
- (52) **U.S. Cl.**
- CPC ..... *C10N 2230/40* (2013.01); *C10N 2230/42* 4,298,486 A 11/1981 Horodysky et al.  
 (2013.01); *C10N 2230/54* (2013.01); *C10N* 4,328,113 A 5/1982 Horodysky et al.  
*2240/10* (2013.01); *C10N 2260/14* (2013.01) 4,367,352 A 1/1983 Watts, Jr. et al.  
 4,370,248 A 1/1983 Horodysky et al.  
 4,374,032 A 2/1983 Gemmill et al.  
 4,376,712 A 3/1983 Horodysky et al.  
 4,382,006 A 5/1983 Horodysky  
 4,389,322 A 6/1983 Horodysky  
 4,406,802 A 9/1983 Horodysky et al.  
 4,413,156 A 11/1983 Watts, Jr. et al.  
 4,426,305 A 1/1984 Malec  
 4,434,408 A 2/1984 Baba et al.  
 4,454,059 A 6/1984 Pindar et al.

(56) **References Cited**

## U.S. PATENT DOCUMENTS

|             |         |                      |                  |             |                                 |
|-------------|---------|----------------------|------------------|-------------|---------------------------------|
| 2,100,993 A | 11/1937 | Bruson               | 4,472,289 A      | 9/1984      | Horodysky et al.                |
| 2,191,498 A | 2/1940  | Reiff                | 4,478,732 A      | 10/1984     | Horodysky et al.                |
| 2,387,501 A | 10/1945 | Dietrich             | 4,522,734 A      | 6/1985      | Horodysky et al.                |
| 2,501,731 A | 3/1950  | Mertes               | 4,537,692 A      | 8/1985      | Horodysky et al.                |
| 2,616,911 A | 11/1952 | Asseff et al.        | 4,541,941 A      | 9/1985      | Horodysky et al.                |
| 2,655,479 A | 10/1953 | Munday et al.        | 4,568,472 A      | 2/1986      | Horodysky et al.                |
| 2,666,746 A | 1/1954  | Munday et al.        | 4,594,171 A      | 6/1986      | Horodysky et al.                |
| 2,721,877 A | 10/1955 | Popkin et al.        | 4,594,172 A      | 6/1986      | Sie                             |
| 2,721,878 A | 10/1955 | Popkin               | 4,692,257 A      | 9/1987      | Horodysky                       |
| 2,777,874 A | 1/1957  | Asseff et al.        | 4,744,920 A      | 5/1988      | Fischer et al.                  |
| 2,817,693 A | 12/1957 | Koome et al.         | 4,767,551 A      | 8/1988      | Hunt                            |
| 3,036,003 A | 5/1962  | Verdol               | 4,792,410 A      | 12/1988     | Schwind et al.                  |
| 3,087,936 A | 4/1963  | Le Suer              | 4,798,684 A      | 1/1989      | Salomon                         |
| 3,172,892 A | 3/1965  | Le Suer et al.       | 4,827,064 A      | 5/1989      | Wu                              |
| 3,200,107 A | 8/1965  | Le Suer              | 4,827,073 A      | 5/1989      | Wu                              |
| 3,215,707 A | 11/1965 | Rense                | 4,897,178 A      | 1/1990      | Best et al.                     |
| 3,219,666 A | 11/1965 | Norman et al.        | 4,910,355 A      | 3/1990      | Shubkin et al.                  |
| 3,250,715 A | 5/1966  | Wyman                | 4,921,594 A      | 5/1990      | Miller                          |
| 3,254,025 A | 5/1966  | Le Suer              | 4,943,672 A      | 7/1990      | Hamner et al.                   |
| 3,272,746 A | 9/1966  | Le Suer et al.       | 4,952,739 A      | 8/1990      | Chen                            |
| 3,275,554 A | 9/1966  | Wagenaar             | 4,956,122 A      | 9/1990      | Watts et al.                    |
| 3,320,162 A | 5/1967  | Axe et al.           | 4,975,177 A      | 12/1990     | Garwood et al.                  |
| 3,322,670 A | 5/1967  | Burt et al.          | 5,055,174 A      | 10/1991     | Howell et al.                   |
| 3,329,658 A | 7/1967  | Fields               | 5,068,487 A      | 11/1991     | Theriot                         |
| 3,316,177 A | 8/1967  | Dorer, Jr.           | 5,084,197 A      | 1/1992      | Galic et al.                    |
| 3,341,542 A | 9/1967  | Le Suer et al.       | 5,354,485 A      | 10/1994     | Tipton et al.                   |
| 3,382,291 A | 5/1968  | Brennan              | 5,430,105 A      | 7/1995      | Redpath et al.                  |
| 3,384,585 A | 5/1968  | Gragson et al.       | 5,641,731 A      | 6/1997      | Baumgart et al.                 |
| 3,413,347 A | 11/1968 | Worrel               | 5,705,458 A      | 1/1998      | Roby et al.                     |
| 3,438,757 A | 4/1969  | Honnen et al.        | 6,034,039 A      | 3/2000      | Gomes et al.                    |
| 3,444,170 A | 5/1969  | Norman et al.        | 6,080,301 A      | 6/2000      | Berlowitz et al.                |
| 3,449,250 A | 6/1969  | Fields               | 6,090,989 A      | 7/2000      | Trewella et al.                 |
| 3,454,555 A | 7/1969  | van der Voort et al. | 6,165,949 A      | 12/2000     | Berlowitz et al.                |
| 3,454,607 A | 7/1969  | Le Suer et al.       | 6,323,164 B1     | 11/2001     | Liesen et al.                   |
| 3,488,284 A | 1/1970  | LeSuer et al.        | 6,774,091 B2     | 8/2004      | Dituro et al.                   |
| 3,519,565 A | 7/1970  | Coleman              | 6,777,378 B2     | 8/2004      | Abraham et al.                  |
| 3,541,012 A | 11/1970 | Stuebe               | 6,887,835 B1     | 5/2005      | Migdal et al.                   |
| 3,565,804 A | 2/1971  | Honnen et al.        | 7,040,930 B2     | 4/2010      | Deckman et al.                  |
| 3,595,791 A | 7/1971  | Cohen                | 8,048,833 B2     | 11/2011     | Habeeb et al.                   |
| 3,629,109 A | 12/1971 | Gergel et al.        | 2003/0119682 A1  | 6/2003      | Saini et al.                    |
| 3,630,904 A | 12/1971 | Musser et al.        | 2007/0155631 A1* | 7/2007      | Muir ..... C07F 5/04<br>508/185 |
| 3,632,511 A | 1/1972  | Liao                 | 2008/0020950 A1  | 1/2008      | Gray et al.                     |
| 3,652,616 A | 3/1972  | Watson et al.        | 2008/0020952 A1  | 1/2008      | Yagishita                       |
| 3,666,730 A | 5/1972  | Coleman              | 2008/0096776 A1  | 4/2008      | Carrick et al.                  |
| 3,687,849 A | 8/1972  | Abbott               | 2008/0261838 A1  | 10/2008     | Karol et al.                    |
| 3,697,574 A | 10/1972 | Piasek et al.        | 2009/0186784 A1  | 7/2009      | Diggs et al.                    |
| 3,702,300 A | 11/1972 | Coleman              | 2014/0106998 A1  | 4/2014      | Nelson et al.                   |
| 3,703,536 A | 11/1972 | Piasek et al.        | EP               | 0464546 A1  | 6/1991                          |
| 3,704,308 A | 11/1972 | Piasek et al.        | EP               | 0464547 A1  | 6/1991                          |
| 3,725,277 A | 4/1973  | Worrel               | EP               | 0471071 B1  | 8/1995                          |
| 3,725,480 A | 4/1973  | Traise et al.        | GB               | 1350257 A   | 4/1974                          |
| 3,726,832 A | 4/1973  | Traise et al.        | GB               | 1390359 A   | 4/1975                          |
| 3,742,082 A | 6/1973  | Brennan              | GB               | 1429494 A   | 3/1976                          |
| 3,751,365 A | 8/1973  | Piasek et al.        | GB               | 1440230 A   | 6/1976                          |
| 3,755,433 A | 8/1973  | Miller et al.        | WO               | 88/03144 A1 | 5/1988                          |
| 3,756,953 A | 9/1973  | Piasek et al.        |                  |             |                                 |
| 3,769,363 A | 10/1973 | Brennan              |                  |             |                                 |
| 3,787,374 A | 1/1974  | Adams                |                  |             |                                 |
| 3,798,165 A | 3/1974  | Piasek et al.        |                  |             |                                 |
| 3,803,039 A | 4/1974  | Piasek et al.        |                  |             |                                 |
| 3,822,209 A | 7/1974  | Knapp et al.         |                  |             |                                 |
| 3,876,720 A | 4/1975  | Heilman et al.       |                  |             |                                 |
| 3,948,800 A | 4/1976  | Meinhardt            |                  |             |                                 |
| 4,100,082 A | 7/1978  | Clason et al.        |                  |             |                                 |
| 4,149,178 A | 4/1979  | Estes                |                  |             |                                 |
| 4,218,330 A | 8/1980  | Shubkin              |                  |             |                                 |

## FOREIGN PATENT DOCUMENTS

(56)

**References Cited**

FOREIGN PATENT DOCUMENTS

WO 96/06904 A1 3/1996  
WO 2016/191409 A1 12/2016

OTHER PUBLICATIONS

Adeka, "Lubricants Additives", [www.adeka.co.jp](http://www.adeka.co.jp), 2013, XP002770253.

Vanderbilt Chemicals, LLC, "Specification MOLYVAN 807 Friction Reducer/Antiwear Compound", [www.rtvanderbiltholding.com](http://www.rtvanderbiltholding.com), 2009, XP002770254.

\* cited by examiner

Fig. 1

|                                                  | 12-83567              | 13-83873  | 13-84096  | 14-38821  | 13-83796  |
|--------------------------------------------------|-----------------------|-----------|-----------|-----------|-----------|
|                                                  | Comparative Example 1 | Example 1 | Example 2 | Example 3 | Example 4 |
| Monoester                                        | 20                    | 20        | 20        | 20        | 20        |
| Other Synthetic Base oil and Viscosity Modifier  | 68.5                  | 68.18     | 67.692    | 68.674    | 67.76     |
| Molyvan I (Moly/Sulfur Ratio: 1/1.4, w/w)        | 1.7                   | 1.22      | 1.708     |           |           |
| Sakura-Lube 300 (Moly/Sulfur Ratio: 1/1.07, w/w) |                       |           |           | 1.526     | 2.44      |
| Mixture of 2ndary ZDDPs                          | 1.2                   | 1.2       | 1.2       | 1.2       | 1.2       |
| Other Additives                                  | 8.6                   | 8.6       | 8.6       | 8.6       | 8.6       |
| VANLUBE 289                                      |                       | 0.8       | 0.8       |           |           |
| PX-3871                                          |                       |           |           |           |           |
|                                                  | 100                   | 100       | 100       | 100       | 100       |
| ASTM D130, 150C, 3 Hrs                           | 48                    | 2C        | 3B        | 1A        | 1A        |
| ASTM D5185 BORON, PPM                            | 250                   | 330       | 320       | 240       | 240       |
| ASTM D5185 CALCIUM, PPM                          | 1630                  | 1680      | 1650      | 1670      | 1630      |
| ASTM D5185 MAGNESIUM, PPM                        | 7.8                   | 3.4       | 3.3       | 8         | 3.4       |
| ASTM D5185 MOLYBDENUM, PPM                       | 1400                  | 1000      | 1400      | 1400      | 2200      |
| ASTM D5185 PHOSPHORUS, PPM                       | 2230                  | 1890      | 2140      | 1630      | 2010      |
| ASTM D5185 ZINC, PPM                             | 1350                  | 1290      | 1300      | 1320      | 1340      |
| MTM Friction Coefficient (140C)                  | 0.058                 | 0.03      | 0.029     | 0.049     | 0.046     |

Fig. 1 (Cont.)

|                                                  | 13-83734  | 14-50150  | 14-38831  | 14-49893  |
|--------------------------------------------------|-----------|-----------|-----------|-----------|
|                                                  | Example 5 | Example 6 | Example 7 | Example 8 |
| Monoester                                        | 20        | 20        | 20        | 20        |
| Other Synthetic Base oil and Viscosity Modifier  | 67.066    | 67.148    | 67.874    | 69.037    |
| Mohyan L (Moly/Sulfur Ratio: 1/1.4, w/w)         | 3.134     | 3.05      | 1.526     | 0.763     |
| Sakura-Tube 300 (Moly/Sulfur Ratio: 1/1.07, w/w) | 1.2       | 1.2       | 1.2       | 1.2       |
| Mixture of 2ndary ZDDPs                          | 8.6       | 8.6       | 8.6       | 8.6       |
| Other Additives                                  |           |           | 0.8       | 0.4       |
| VANLUBE 289                                      |           |           |           |           |
| PX-3871                                          |           |           |           |           |
|                                                  | 100       | 100       | 100       | 100       |
| ASTM D130, 150C, 3 Hrs                           | 1A        | 1A        | 1A        | 1A        |
| ASTM D5185 BORON, PPM                            | 240       | 230       | 320       | 280       |
| ASTM D5185 CALCIUM, PPM                          | 1630      | 1630      | 1660      | 1640      |
| ASTM D5185 MAGNESIUM, PPM                        | 3.1       | 4.4       | 8.1       | 3.9       |
| ASTM D5185 MOLYBDENUM, PPM                       | 2800      | 2800      | 1400      | 690       |
| ASTM D5185 PHOSPHORUS, PPM                       | 2150      | 2080      | 1630      | 1370      |
| ASTM D5185 ZINC, PPM                             | 1260      | 1250      | 1310      | 1260      |
| MM Friction Coefficient (140C)                   | 0.046     | 0.043     | 0.031     | 0.038     |

Fig. 1 (Cont.)

|                                                  | 14-46486              | 14-50148              | 15-67870              | 15-67956              |
|--------------------------------------------------|-----------------------|-----------------------|-----------------------|-----------------------|
|                                                  | Comparative Example 2 | Comparative Example 3 | Comparative Example 4 | Comparative Example 5 |
| Monooester                                       | 20                    | 20                    | 20                    | 20                    |
| Other Synthetic Base oil and Viscosity Modifier  | 69.4                  | 68.6                  | 67.492                | 67.674                |
| Molyvan L (Moly/Sulfur Ratio: 1/1.4, w/w)        |                       |                       | 1.708                 |                       |
| Sakura-Lube 300 (Moly/Sulfur Ratio: 1/1.07, w/w) | 1.2                   | 1.2                   | 1.2                   | 1.2                   |
| Mixture of 2ndary ZDDPs                          |                       |                       |                       | 1.526                 |
| Other Additives                                  | 8.6                   | 8.6                   | 8.6                   | 8.6                   |
| VANLUBE 289                                      | 0.8                   | 1.6                   |                       |                       |
| PX-3871                                          |                       |                       | 1.0                   | 1.0                   |
|                                                  | 100                   | 100                   | 100                   | 100                   |
| ASTM D130, 150C, 3 Hrs                           | 1A                    | 1A                    | 3B                    | 1B                    |
| ASTM D5185 BORON, PPM                            | 310                   | 390                   | 860                   | 870                   |
| ASTM D5185 CALCIUM, PPM                          | 1620                  | 1660                  | 1670                  | 1670                  |
| ASTM D5185 MAGNESIUM, PPM                        | 3.56                  | 3.72                  | 7.7                   | 7.71                  |
| ASTM D5185 MOLYBDENUM, PPM                       | 0.54                  | 1.2                   | 1400                  | 1400                  |
| ASTM D5185 PHOSPHORUS, PPM                       | 1110                  | 1120                  | 2080                  | 1570                  |
| ASTM D5185 ZINC, PPM                             | 1260                  | 1250                  | 1200                  | 1250                  |
| MTM Friction Coefficient (140C)                  | 0.094                 | 0.092                 | 0.062                 | 0.054                 |

Fig. 2

|                                           | 14-79866  | 13078485   | 13077598              | 13088901              |
|-------------------------------------------|-----------|------------|-----------------------|-----------------------|
|                                           | Example 9 | Example 10 | Comparative Example 6 | Comparative Example 7 |
| Synthetic Base oil and Viscosity Modifier | 79.86     | 79.7       | 80.66                 | 80.58                 |
| Molyvan L                                 | 1.22      | 1.22       | 1.22                  | 1.22                  |
| Mixture of Primary and Secondary ZDDPs    | 2.1       | 2.1        | 2.1                   | 2.1                   |
| Other Additives                           | 14.72     | 14.72      | 14.72                 | 14.72                 |
| IRGAMET 39                                |           | 0.08       |                       | 0.08                  |
| HITEC 4313                                |           | 0.08       |                       |                       |
| VANLUBE 7723                              |           |            |                       |                       |
| Borated Dispersant                        | 1.3       | 1.3        | 1.3                   | 1.3                   |
| VANLUBE 289                               | 0.8       | 0.8        |                       |                       |
| PX-3871                                   |           |            |                       |                       |
| ASTM D130, 150 C, 3 Hrs                   | 100       | 100        | 100                   | 100                   |
| ASTM D5185 BORON, PPM                     | 2B        | 2A         | 4B                    | 4A                    |
| ASTM D5185 CALCIUM, PPM                   | 180       | 190        | 100                   | 100                   |
| ASTM D5185 MAGNESIUM, PPM                 | 1150      | 1080       | 1090                  | 1150                  |
| ASTM D5185 MOLYBDENUM, PPM                | 877       | 808        | 812                   | 856                   |
| ASTM D5185 PHOSPHORUS, PPM                | 2440      | 2510       | 2530                  | 2420                  |
| ASTM D5185 ZINC, PPM                      | 1970      | 2070       | 2060                  | 2010                  |
| MTM Friction Coefficient                  | 0.029     | 0.059      | 0.069                 | 0.069                 |

Fig. 2 (Cont.)

|                                           | 13089028              | 13089701              | 13078907               | 13078241               |
|-------------------------------------------|-----------------------|-----------------------|------------------------|------------------------|
|                                           | Comparative Example 8 | Comparative Example 9 | Comparative Example 10 | Comparative Example 11 |
| Synthetic Base oil and Viscosity Modifier | 80.5                  | 79.36                 | 80.58                  | 80.5                   |
| Molyvan L                                 | 1.22                  | 1.22                  | 1.22                   | 1.22                   |
| Mixture of Primary and Secondary ZDDPs    | 2.1                   | 2.1                   | 2.1                    | 2.1                    |
| Other Additives                           | 14.72                 | 14.72                 | 14.72                  | 14.72                  |
| IRGAMET 39                                |                       |                       |                        | 0.08                   |
| HITEC 4313                                |                       |                       | 0.08                   | 0.08                   |
| VANLUBE 7723                              | 0.16                  |                       |                        |                        |
| Borated Dispersant                        | 1.3                   | 2.6                   | 1.3                    | 1.3                    |
| VANLUBE 289                               |                       |                       |                        |                        |
| PX-3871                                   |                       |                       |                        |                        |
| ASTM D130, 150 C, 3 HRS                   | 100                   | 100                   | 100                    | 100                    |
| ASTM D5185 BORON, PPM                     | 4B                    | 4B                    | 4B                     | 4B                     |
| ASTM D5185 CALCIUM, PPM                   | 100                   | 210                   | 110                    | 100                    |
| ASTM D5185 MAGNESIUM, PPM                 | 1130                  | 1150                  | 1080                   | 1110                   |
| ASTM D5185 MOLYBDENUM, PPM                | 845                   | 815                   | 812                    | 867                    |
| ASTM D5185 PHOSPHORUS, PPM                | 1000                  | 1000                  | 1000                   | 990                    |
| ASTM D5185 ZINC, PPM                      | 2440                  | 2470                  | 2510                   | 2520                   |
| MTM Friction Coefficient                  | 0.065                 | 0.065                 | 0.049                  | 0.052                  |

Fig. 2 (Cont.)

|                                           | 13078460               | 13084929               | 15-69097               |
|-------------------------------------------|------------------------|------------------------|------------------------|
|                                           | Comparative Example 12 | Comparative Example 13 | Comparative Example 14 |
| Synthetic Base oil and Viscosity Modifier | 80.34                  | 79.2                   | 79.66                  |
| Molyvan L                                 | 1.22                   | 1.22                   | 1.22                   |
| Mixture of Primary and Secondary ZDDPs    | 2.1                    | 2.1                    | 2.1                    |
| Other Additives                           | 14.72                  | 14.72                  | 14.72                  |
| IRGAMET 39                                | 0.08                   | 0.08                   |                        |
| HITEC 4313                                | 0.08                   | 0.08                   |                        |
| VANLUBE 7723                              | 0.16                   |                        |                        |
| Borated Dispersant                        | 1.3                    | 2.6                    | 1.3                    |
| VANLUBE 289                               |                        |                        |                        |
| PX-3871                                   |                        |                        | 1.0                    |
| ASTM D130, 150 C, 3 Hrs                   | 100                    | 100                    | 100                    |
| ASTM D5185 BORON, PPM                     | 4A                     | 4B                     | 4B                     |
| ASTM D5185 CALCIUM, PPM                   | 1080                   | 1140                   | 1140                   |
| ASTM D5185 MAGNESIUM, PPM                 | 813                    | 809                    | 809                    |
| ASTM D5185 MOLYBDENUM, PPM                | 1000                   | 990                    | 990                    |
| ASTM D5185 PHOSPHORUS, PPM                | 2480                   | 2440                   | 2440                   |
| ASTM D5185 ZINC, PPM                      | 2030                   | 2010                   | 2010                   |
| MHM Friction Coefficient                  | 0.066                  | 0.046                  | 0.046                  |

Fig. 3

|                             | Comparative | Example 1 | Example 1 | Example 2 | Example 3 | Example 4 | Example 5 | Example 6 | Example 7 |
|-----------------------------|-------------|-----------|-----------|-----------|-----------|-----------|-----------|-----------|-----------|
| Comparative                 |             |           |           |           |           |           |           |           |           |
| Example 1                   | 12-83567    | 13-83873  | 13-84096  | 14-38821  | 13-83796  | 13-83734  | 13-83734  | 14-38831  | 14-38831  |
| Molybdenum, ppm             | 1400        | 1000      | 1400      | 1400      | 2200      | 2800      | 2800      | 1400      | 1400      |
| MoDTP, Moly/Sulfur Ratio    | 1:1.4       | 1:1.4     | 1:1.4     | 1:1.07    | 1:1.07    | 1:1.07    | 1:1.07    | 1:1.07    | 1:1.07    |
| Vanlube 289, Wt%            | 0           | 0.8       | 0.8       | 0         | 0         | 0         | 0         | 0.8       | 0.8       |
| ASTM D130 at 150°C (3hr.)   | 4B          | 2C        | 3B        | 1A        | 1A        | 1A        | 1A        | 1A        | 1A        |
| Friction Coefficient (140C) | 0.058       | 0.030     | 0.029     | 0.049     | 0.046     | 0.046     | 0.046     | 0.031     | 0.031     |

Fig. 4

|                                                          | 13-084396     | 13-084525     |
|----------------------------------------------------------|---------------|---------------|
|                                                          | Example<br>11 | Example<br>12 |
| Monoester                                                | 20.00         | 20.00         |
| Other Synthetic Base oil and Viscosity Modifier          | 66.47         | 67.47         |
| Sakura-Lube 300 (Moly/Sulfur Ratio: 1/1.07, w/w)         | 1.526         | 1.526         |
| Mixture of 2ndary ZDDPs                                  | 1.2           | 1.2           |
| Other Additives                                          | 9.8           | 9.8           |
| VANLUBE 289                                              | 1.0           | 0.0           |
|                                                          | 100.00        | 100.00        |
| ASTM D130, 150C, 3 Hrs                                   | 1A            | 1A            |
| ASTM D5185 of Used Oil from ASTM D130, 150C, COPPER, PPM | 7.5           | 9.1           |
| ASTM D5185 BORON, PPM                                    | 340           | 230           |
| ASTM D5185 CALCIUM, PPM                                  | 1680          | 1650          |
| ASTM D5185 MAGNESIUM, PPM                                | 3.4           | 3.3           |
| ASTM D5185 MOLYBDENUM, PPM                               | 1400          | 1400          |
| ASTM D5185 PHOSPHORUS, PPM                               | 1710          | 1630          |
| ASTM D5185 ZINC, PPM                                     | 1340          | 1260          |
| MTM Friction Coefficient (140C)                          | 0.032         | 0.042         |
| D130 USED OIL                                            | 13-087444     | 13-087445     |

Fig. 5

| Class | Designation      | Description                                                                                                                                 |
|-------|------------------|---------------------------------------------------------------------------------------------------------------------------------------------|
| 1     | Slight Tarnish   | 1a Light orange, almost the same as a freshly polished strip<br>1b Dark Orange                                                              |
| 2     | Moderate Tarnish | 2a Claret Red<br>2b Lavander<br>2c Multi-colored with lavender blue and/or silver overlaid on claret red<br>2d Silvery<br>2e Brassy or gold |
| 3     | Dark Tarnish     | 3a Magenta overcast on brassy strip<br>3b Multicolored with red and green showing (peacock), but no gray                                    |
| 4     | Corrosion        | 4a Transparent black, dark gray or brown with peacock green barely showing<br>4b Graphite or lusterless black<br>4c Glassy or jet black     |

## 1

## LUBRICANT COMPOSITIONS

## FIELD

This disclosure relates to a method for improving corrosion protection and friction coefficient in an engine or other mechanical component lubricated with a lubricating oil. This disclosure also relates to lubricating oils that are useful in internal combustion engines.

## BACKGROUND

Lubrication involves the process of friction reduction, accomplished by maintaining a film of a lubricant between surfaces which are moving with respect to each other. The lubricant prevents contact of the moving surfaces, thus greatly lowering the coefficient of friction. In addition to this function, the lubricant also can be called upon to perform heat removal, containment of contaminants, and other important functions. Additives have been developed to establish or enhance various properties of lubricants. Various additives which are used include viscosity improvers, detergents, dispersants, antioxidants, extreme pressure additives, and corrosion inhibitors.

Fuel efficiency is one of the most challenging areas in today's lubricant development. Friction modifiers are widely used in lubricant formulations. Organic molybdenum compounds are very effective friction modifiers. However, corrosion is one of the main factors that limit the broad use of high concentrations of organic molybdenum compounds.

There are two commonly used organic molybdenum compound friction modifiers, namely molybdenum dialkyldithiocarbamate (MoDTC) and molybdenum dialkyldithiophosphate (MoDTP). It is also known that these molybdenum compounds contribute to copper corrosion. See, for example, EP 0316610A1 and R. T. Vanderbilt literatures that indicate in some formulations, the presence of Molyvan™ 822 (MoDTC) and Molyvan™ L (MoDTP) contribute to copper corrosion which is detrimental to some diesel engines. The corrosion issue is one of the key factors that limit the use of high concentration of organic molybdenum compounds in formulating high fuel economy lubricants.

Despite advances in lubricant oil formulation technology, there exists a need for an engine oil lubricant that effectively improves corrosion protection and friction coefficient in order to improve engine durability and fuel efficiency.

## SUMMARY

This disclosure relates to a method for improving corrosion protection and friction coefficient in an engine or other mechanical component lubricated with a lubricating oil by using as the lubricating oil a formulated oil. The formulated oil has a composition comprising a lubricating oil base stock as a major component, and a mixture of (i) at least one organic molybdenum compound, and (ii) at least one borated ester, as a minor component. Corrosion protection and friction coefficient are improved and fuel efficiency is maintained or improved as compared to corrosion protection, friction coefficient and fuel efficiency achieved using a lubricating oil containing a minor component other than the mixture of (i) at least one organic molybdenum compound, and (ii) at least one borated ester.

This disclosure also relates in part to a method for improving corrosion protection and friction coefficient in an engine or other mechanical component lubricated with a lubricating oil by using as the lubricating oil a formulated

## 2

oil. The formulated oil has a composition comprising a lubricating oil base stock as a major component, and at least one low sulfur organic molybdenum compound having a molybdenum to sulfur ratio from about 1 to less than about 1.1, as a minor component. Corrosion protection and friction coefficient are improved and fuel efficiency is maintained or improved as compared to corrosion protection, friction coefficient and fuel efficiency achieved using a lubricating oil containing a minor component other than the low sulfur organic molybdenum compound having a molybdenum to sulfur ratio from about 1 to less than about 1.1.

This disclosure further relates in part to a method for improving corrosion protection and friction coefficient in an engine or other mechanical component lubricated with a lubricating oil by using as the lubricating oil a formulated oil. The formulated oil has a composition comprising a lubricating oil base stock as a major component, and at least one low sulfur molybdenum dithiophosphate having a molybdenum to sulfur ratio from about 1 to less than about 1.1, as a minor component. Corrosion protection and friction coefficient are improved and fuel efficiency is maintained or improved as compared to corrosion protection, friction coefficient and fuel efficiency achieved using a lubricating oil containing a minor component other than the low sulfur molybdenum dithiophosphate having a molybdenum to sulfur ratio from about 1 to less than about 1.1.

This disclosure yet further relates in part to a method for improving corrosion protection and friction coefficient in an engine or other mechanical component lubricated with a lubricating oil by using as the lubricating oil a formulated oil. The formulated oil has a composition comprising a lubricating oil base stock as a major component, and a mixture of (i) at least one low sulfur molybdenum dithiophosphate having a molybdenum to sulfur ratio from about 1 to less than about 1.1, and (ii) at least one borated ester, as a minor component. Corrosion protection and friction coefficient are improved and fuel efficiency is maintained or improved as compared to corrosion protection, friction coefficient and fuel efficiency achieved using a lubricating oil containing a minor component other than the mixture of (i) at least one low sulfur molybdenum dithiophosphate having a molybdenum to sulfur ratio from about 1 to less than about 1.1, and (ii) at least one borated ester.

This disclosure relates to a lubricating oil having a composition comprising a lubricating oil base stock as a major component, and a mixture of (i) at least one organic molybdenum compound, and (ii) at least one borated ester, as a minor component. Corrosion protection and friction coefficient are improved and fuel efficiency is maintained or improved in an engine or other mechanical component lubricated with the lubricating oil, as compared to corrosion protection, friction coefficient and fuel efficiency achieved using a lubricating oil containing a minor component other than the mixture of (i) at least one organic molybdenum compound, and (ii) at least one borated ester.

This disclosure also relates in part to a lubricating oil having a composition comprising a lubricating oil base stock as a major component, and at least one low sulfur organic molybdenum compound having a molybdenum to sulfur ratio from about 1 to less than about 1.1, as a minor component. Corrosion protection and friction coefficient are improved and fuel efficiency is maintained or improved in an engine or other mechanical component lubricated with the lubricating oil, as compared to corrosion protection, friction coefficient and fuel efficiency achieved using a lubricating oil containing a minor component other than the low sulfur

organic molybdenum compound having a molybdenum to sulfur ratio from about 1 to less than about 1.1.

This disclosure further relates in part to a lubricating oil having a composition comprising a lubricating oil base stock as a major component, and at least one low sulfur molybdenum dithiophosphate having a molybdenum to sulfur ratio from about 1 to less than about 1.1, as a minor component. Corrosion protection and friction coefficient are improved and fuel efficiency is maintained or improved in an engine or other mechanical component lubricated with the lubricating oil, as compared to corrosion protection, friction coefficient and fuel efficiency achieved using a lubricating oil containing a minor component other than the low sulfur molybdenum dithiophosphate having a molybdenum to sulfur ratio from about 1 to less than about 1.1.

This disclosure yet further relates in part to a lubricating oil having a composition comprising a lubricating oil base stock as a major component, and a mixture of (i) at least one low sulfur molybdenum dithiophosphate having a molybdenum to sulfur ratio from about 1 to less than about 1.1, and (ii) at least one borated ester, as a minor component. Corrosion protection and friction coefficient are improved and fuel efficiency is maintained or improved in an engine or other mechanical component lubricated with the lubricating oil, as compared to corrosion protection, friction coefficient and fuel efficiency achieved using a lubricating oil containing a minor component other than the mixture of (i) at least one low sulfur molybdenum dithiophosphate having a molybdenum to sulfur ratio from about 1 to less than about 1.1, and (ii) at least one borated ester.

It has been surprisingly found that, in a lubricant formulation containing 1000 ppm or higher molybdenum, copper corrosion can be mitigated by addition of borated ester (e.g., Vanlube<sup>TM</sup> 289) or by use of low sulfur molybdenum dithiophosphate having a molybdenum to sulfur ratio of 1:1.07 (e.g., Sakura-Lube<sup>TM</sup> 300). In addition, a synergistic effect was observed between low sulfur molybdenum dithiophosphate having a molybdenum to sulfur ratio of 1:1.07 (e.g., Sakura-Lube<sup>TM</sup> 300) and a borated ester (e.g., Vanlube<sup>TM</sup> 289) in friction reduction (see, for example, FIG. 1).

Other objects and advantages of the present disclosure will become apparent from the detailed description that follows.

#### BRIEF DESCRIPTION OF THE DRAWINGS

FIG. 1 shows formulations prepared in accordance with the Examples, and the results of MTM testing and copper corrosion testing in accordance with the Examples. In particular, FIG. 1 shows the effects of borated ester (Vanlube<sup>TM</sup> 289), low sulfur molybdenum dithiophosphate having a molybdenum to sulfur ratio of 1:1.07 (Sakura-Lube<sup>TM</sup> 300), and low sulfur molybdenum dithiophosphate having a molybdenum to sulfur ratio of 1:1.4 (Molyvan<sup>TM</sup> L) on copper corrosion and friction coefficients of molybdenum-containing formulations.

FIG. 2 shows formulations prepared in accordance with the Examples, and the results of MTM testing and copper corrosion testing in accordance with the Examples. In particular, FIG. 2 shows a comparison of various additives, including corrosion inhibitors, versus borated ester (Vanlube<sup>TM</sup> 289) on copper corrosion and friction coefficients of molybdenum-containing formulations.

FIG. 3 shows selected formulations of FIG. 1, and the results of MTM testing and copper corrosion testing of the selected formulations. FIG. 3 shows pictures of copper strips used in the copper corrosion testing in accordance with

ASTM D130. FIG. 3 shows that in a lubricant formulation containing 1000 ppm or higher molybdenum, copper corrosion was mitigated by addition of borated ester (Vanlube<sup>TM</sup> 289) (marketed as an antiwear/antscuff additive and friction reducer) or by use of 1 low sulfur molybdenum dithiophosphate having a molybdenum to sulfur ratio of 1:1.07 (Sakura-Lube<sup>TM</sup> 300).

FIG. 4 shows formulations prepared in accordance with the Examples, and the results of MTM testing and copper corrosion testing in accordance with the Examples. In particular, FIG. 4 shows wear metals in used lubricants. The determination of wear metals, contaminants and selected elements in used lubricating oils was conducted in accordance with ASTM D5185.

FIG. 5 shows a standard chart for comparing results of corrosion protection testing by a copper strip corrosion test in accordance with ASTM D130. The test evaluates the degree to which a lubricant will corrode copper-containing materials (e.g., bronze and brass).

#### DETAILED DESCRIPTION

All numerical values within the detailed description and the claims herein are modified by “about” or “approximately” the indicated value, and take into account experimental error and variations that would be expected by a person having ordinary skill in the art.

It has now been found that improved corrosion protection and friction coefficient can be attained in an engine or other mechanical component lubricated with a lubricating oil by using as the lubricating oil a formulated oil that has a mixture of (i) at least one organic molybdenum compound, and (ii) at least one borated ester, in the lubricating oil. The formulated oil preferably comprises a lubricating oil base stock as a major component, and a mixture of (i) at least one organic molybdenum compound, and (ii) at least one borated ester, as a minor component. The lubricating oils of this disclosure are particularly advantageous as passenger vehicle engine oil (PVEO) products.

It has also been found that improved corrosion protection and friction coefficient can be attained in an engine or other mechanical component lubricated with a lubricating oil by using as the lubricating oil a formulated oil that has at least one low sulfur organic molybdenum compound having a molybdenum to sulfur ratio from about 1 to less than about 1.1, in the lubricating oil. The formulated oil preferably comprises a lubricating oil base stock as a major component, and at least one low sulfur organic molybdenum compound having a molybdenum to sulfur ratio from about 1 to less than about 1.1, as a minor component.

It has further been found that improved corrosion protection and friction coefficient can be attained in an engine or other mechanical component lubricated with a lubricating oil by using as the lubricating oil a formulated oil that has at least one low sulfur molybdenum dithiophosphate having a molybdenum to sulfur ratio from about 1 to less than about 1.1, in the lubricating oil. The formulated oil preferably comprises a lubricating oil base stock as a major component, and at least one low sulfur molybdenum dithiophosphate having a molybdenum to sulfur ratio from about 1 to less than about 1.1, as a minor component.

It has yet further been found that improved corrosion protection and friction coefficient can be attained in an engine or other mechanical component lubricated with a lubricating oil by using as the lubricating oil a formulated oil that has a mixture of (i) at least one low sulfur molybdenum dithiophosphate having a molybdenum to sulfur ratio from

about 1 to less than about 1.1, and (ii) at least one borated ester, in the lubricating oil. The formulated oil preferably comprises a lubricating oil base stock as a major component, and a mixture of (i) at least one low sulfur molybdenum dithiophosphate having a molybdenum to sulfur ratio from about 1 to less than about 1.1, and (ii) at least one borated ester, as a minor component.

The present disclosure provides lubricant compositions with excellent corrosion protection and antiwear properties. Antiwear additives are generally required for reducing wear in operating equipment where two solid surfaces engage in contact. In the absence of antiwear chemistry, the surfaces can rub together causing material loss on one or both surfaces which can eventually lead to equipment malfunction and failure. Antiwear additives can produce a protective surface layer which reduces wear and material loss. Most commonly the materials of interest are metals such as steel and other iron-containing alloys. However, other materials such as ceramics, polymer coatings, diamond-like carbon, corresponding composites, and the like can also be used to produce durable surfaces in modern equipment. The lubricant compositions of this disclosure can provide antiwear properties to such surfaces.

The lubricant compositions of this disclosure provide advantaged corrosion protection and wear, including advantaged wear and friction, performance in the lubrication of internal combustion engines, power trains, drivelines, transmissions, gears, gear trains, gear sets, compressors, pumps, hydraulic systems, bearings, bushings, turbines, and the like.

Also, the lubricant compositions of this disclosure provide advantaged corrosion protection and wear, including advantaged wear and friction, performance in the lubrication of mechanical components, which can include, for example, pistons, piston rings, cylinder liners, cylinders, cams, tappets, lifters, bearings (journal, roller, tapered, needle, ball, and the like), gears, valves, and the like.

Further, the lubricant compositions of this disclosure provide advantaged corrosion protection and wear, including advantaged wear and friction, performance as a component in lubricant compositions, which can include, for example, lubricating liquids, semi-solids, solids, greases, dispersions, suspensions, material concentrates, additive concentrates, and the like.

The lubricant compositions of this disclosure are useful in additive concentrates that include the combination of the minor component of this disclosure with at least one other additive component, having combined weight % concentrations in the range of 1% to 80%, preferably 1% to 60%, more preferably 1% to 50%, even more preferably 1% to 40%, and in some instances preferably 1% to 30%. Under some circumstances, the combined weight % concentrations cited above may be in the range of 1% to 20%, and preferably 1% to 10%.

Yet further, the lubricant compositions of this disclosure provide advantaged corrosion protection and wear, including advantaged wear and friction, performance under diverse lubrication regimes, that include, for example, hydrodynamic, elastohydrodynamic, boundary, mixed lubrication, extreme pressure regimes, and the like.

The lubricant compositions of this disclosure provide advantaged corrosion protection and wear, including advantaged wear and friction, performance under a range of lubrication contact pressures, less than 1 MPa, and from 1 MPa to greater than 10 GPa, preferably greater than 10 MPa, more preferably greater than 100 MPa, even more preferably greater than 300 MPa. Under certain circumstances, the lubricant compositions of this disclosure pro-

vide advantaged corrosion protection and wear, including advantaged wear and friction, performance at greater than 0.5 GPa, often at greater than 1 GPa, sometimes greater than 2 GPa, under selected circumstances greater than 5 GPa.

Also, the lubricant compositions of this disclosure provide advantaged wear, including advantaged corrosion protection and wear and friction, performance in spark-ignition internal combustion engines, compression-ignition internal combustion engines, mixed-ignition (spark-assisted and compression) internal combustion engines, jet- or plasma-ignition internal combustion engines, and the like.

Further, the lubricant compositions of this disclosure provide advantaged corrosion protection and wear, including advantaged wear and friction, performance in diverse engine and power plant types, which can include, for example, the following: 2-stroke engines; 4-stroke engine; engines with alternate stroke designs greater than 2-stroke, such as 5-stroke, or 7-stroke, and the like; rotary engines; dedicated EGR (exhaust gas recirculation) fueled engines; free-piston type engines; opposable-piston opposable-cylinder type engines; engines that function in hybrid propulsion systems, that can further include electrical-based power systems, hydraulic-based power systems, diverse system designs such as parallel, series, non-parallel, and the like.

Yet further, the lubricant compositions of this disclosure provide advantaged corrosion protection and wear, including advantaged wear and friction, performance in, for example, the following: naturally aspirated engines; turbocharged and supercharged, port-fueled injection engines; turbocharged and supercharged, direct injection engines (for gasoline, diesel, natural gas, mixtures of these, and other fuel types); turbocharged engines designed to operate with in-cylinder combustion pressures of greater than 12 bar, preferably greater than 18 bar, more preferably greater than 20 bar, even more preferably greater than 22 bar, and in certain instances combustion pressures greater than 24 bar, even greater than 26 bar, and even more so greater than 28 bar, and with particular designs greater than 30 bar; engines having low-temperature burn combustion, lean-burn combustion, and high thermal efficiency designs.

Also, the lubricant compositions of this disclosure provide advantaged corrosion protection and wear, including advantaged wear and friction, performance in engines that are fueled with fuel compositions that include, for example, the following: gasoline; distillate fuel, diesel fuel, jet fuel, gas-to-liquid and Fischer-Tropsch-derived high-cetane fuels; compressed natural gas, liquefied natural gas, methane, ethane, propane, other natural gas components, other natural gas liquids; ethanol, methanol, other higher MW alcohols; FAMEs, vegetable-derived esters and polyesters; biodiesel, bio-derived and bio-based fuels; hydrogen; dimethyl ether; other alternate fuels; fuels diluted with EGR (exhaust gas recirculation) gases, with EGR gases enriched in hydrogen or carbon monoxide or combinations of H<sub>2</sub>/CO, in both dilute and high concentration (in concentrations of >0.1%, preferably >0.5%, more preferably >1%, even more preferably >2%, and even more so preferably >3%), and blends or combinations of these in proportions that enhance combustion efficiency, power, cleanliness, anti-knock, and anti-LSPI (low speed pre-ignition).

Further, the lubricant compositions of this disclosure provide advantaged corrosion protection and wear, including advantaged wear and friction, performance on lubricated surfaces that include, for example, the following: metals, metal alloys, non-metals, non-metal alloys, mixed carbon-metal composites and alloys, mixed carbon-nonmetal composites and alloys, ferrous metals, ferrous composites and

alloys, non-ferrous metals, non-ferrous composites and alloys, titanium, titanium composites and alloys, aluminum, aluminum composites and alloys, magnesium, magnesium composites and alloys, ion-implanted metals and alloys, plasma modified surfaces; surface modified materials; coatings; mono-layer, multi-layer, and gradient layered coatings; honed surfaces; polished surfaces; etched surfaces; textured surfaces; micro and nano structures on textured surfaces; super-finished surfaces; diamond-like carbon (DLC), DLC with high-hydrogen content, DLC with moderate hydrogen content, DLC with low-hydrogen content, DLC with near-zero hydrogen content, DLC composites, DLC-metal compositions and composites, DLC-nonmetal compositions and composites; ceramics, ceramic oxides, ceramic nitrides, FeN, CrN, ceramic carbides, mixed ceramic compositions, and the like; polymers, thermoplastic polymers, engineered polymers, polymer blends, polymer alloys, polymer composites; materials compositions and composites containing dry lubricants, that include, for example, graphite, carbon, molybdenum, molybdenum disulfide, polytetrafluoroethylene, polyperfluoropropylene, polyperfluoroalkylethers, and the like.

Yet further, the lubricant compositions of this disclosure provide advantaged corrosion protection and wear, including advantaged wear and friction, performance on lubricated surfaces of 3-D printed materials, and similar materials derived from additive manufacturing techniques, with or without post-printing surface finishing; surfaces of 3-D printed materials that have been post-printing treated with coatings, which may include plasma spray coatings, ion beam-generated coatings, electrolytically- or galvanically-generated coatings, electro-deposition coatings, vapor-deposition coatings, liquid-deposition coatings, thermal coatings, laser-based coatings; surfaces of 3-D printed materials, where the surfaces may be as-printed, finished, or coated, that include: metals, metal alloys, non-metals, non-metal alloys, mixed carbon-metal composites and alloys, mixed carbon-nonmetal composites and alloys, ferrous metals, ferrous composites and alloys, non-ferrous metals, non-ferrous composites and alloys, titanium, titanium composites and alloys, aluminum, aluminum composites and alloys, magnesium, magnesium composites and alloys, ion-implanted metals and alloys; plasma modified surfaces; surface modified materials; mono-layer, multi-layer, and gradient layered coatings; honed surfaces; polished surfaces; etched surfaces; textured surfaces; micro and nano structures on textured surfaces; super-finished surfaces; diamond-like carbon (DLC), DLC with high-hydrogen content, DLC with moderate hydrogen content, DLC with low-hydrogen content, DLC with near-zero hydrogen content, DLC composites, DLC-metal compositions and composites, DLC-nonmetal compositions and composites; ceramics, ceramic oxides, ceramic nitrides, FeN, CrN, ceramic carbides, mixed ceramic compositions, and the like; polymers, thermoplastic polymers, engineered polymers, polymer blends, polymer alloys, polymer composites; materials compositions and composites containing dry lubricants, that include, for example, graphite, carbon, molybdenum, molybdenum disulfide, polytetrafluoroethylene, polyperfluoropropylene, polyperfluoroalkylethers, and the like.

Still further, the lubricant compositions of this disclosure provide advantaged synergistic corrosion protection and wear, including advantaged synergistic wear and friction, performance in combination with one or more performance additives, with performance additives at effective concentration ranges, and with performance additives at effective ratios with the minor component of this disclosure.

#### Lubricating Oil Base Stocks and Co-Base Stocks

A wide range of lubricating base oils is known in the art. Lubricating base oils that are useful in the present disclosure are natural oils, mineral oils and synthetic oils, and unconventional oils (or mixtures thereof) can be used unrefined, refined, or rerefined (the latter is also known as reclaimed or reprocessed oil). Unrefined oils are those obtained directly from a natural or synthetic source and used without added purification. These include shale oil obtained directly from retorting operations, petroleum oil obtained directly from primary distillation, and ester oil obtained directly from an esterification process. Refined oils are similar to the oils discussed for unrefined oils except refined oils are subjected to one or more purification steps to improve at least one lubricating oil property. One skilled in the art is familiar with many purification processes. These processes include solvent extraction, secondary distillation, acid extraction, base extraction, filtration, and percolation. Rerefined oils are obtained by processes analogous to refined oils but using an oil that has been previously used as a feed stock.

Groups I, II, III, IV and V are broad base oil stock categories developed and defined by the American Petroleum Institute (API Publication 1509; [www.API.org](http://www.API.org)) to create guidelines for lubricant base oils. Group I base stocks have a viscosity index of between about 80 to 120 and contain greater than about 0.03% sulfur and/or less than about 90% saturates. Group II base stocks have a viscosity index of between about 80 to 120, and contain less than or equal to about 0.03% sulfur and greater than or equal to about 90% saturates. Group III stocks have a viscosity index greater than about 120 and contain less than or equal to about 0.03% sulfur and greater than about 90% saturates. Group IV includes polyalphaolefins (PAO). Group V base stock includes base stocks not included in Groups I-IV. The table below summarizes properties of each of these five groups.

|           | Base Oil Properties                                               |                        |                 |
|-----------|-------------------------------------------------------------------|------------------------|-----------------|
|           | Saturates                                                         | Sulfur                 | Viscosity Index |
| Group I   | <90 and/or                                                        | >0.03% and             | ≥80 and <120    |
| Group II  | ≥90 and                                                           | ≤0.03% and             | ≥80 and <120    |
| Group III | ≥90 and                                                           | ≤0.03% and             | ≥120            |
| Group IV  |                                                                   | polyalphaolefins (PAO) |                 |
| Group V   | All other base oil stocks not included in Groups I, II, III or IV |                        |                 |

Natural oils include animal oils, vegetable oils (castor oil and lard oil, for example), and mineral oils. Animal and vegetable oils possessing favorable thermal oxidative stability can be used. Of the natural oils, mineral oils are preferred. Mineral oils vary widely as to their crude source, for example, as to whether they are paraffinic, naphthenic, or mixed paraffinic-naphthenic. Oils derived from coal or shale are also useful. Natural oils vary also as to the method used for their production and purification, for example, their distillation range and whether they are straight run or cracked, hydrorefined, or solvent extracted.

Group II and/or Group III hydroprocessed or hydrocracked base stocks are also well known base stock oils.

Synthetic oils include hydrocarbon oil. Hydrocarbon oils include oils such as polymerized and interpolymerized olefins (polybutylenes, polypropylenes, propylene isobutylene copolymers, ethylene-olefin copolymers, and ethylene-alphaolefin copolymers, for example). Polyalphaolefin (PAO) oil base stocks are commonly used synthetic hydrocarbon

oil. By way of example, PAOs derived from C<sub>8</sub>, C<sub>10</sub>, C<sub>12</sub>, C<sub>14</sub> olefins or mixtures thereof may be utilized. See U.S. Pat. Nos. 4,956,122; 4,827,064; and 4,827,073.

The number average molecular weights of the PAOs, which are known materials and generally available on a major commercial scale from suppliers such as ExxonMobil Chemical Company, Chevron Phillips Chemical Company, BP, and others, typically vary from about 250 to about 3,000, although PAO's may be made in viscosities up to about 150 cSt (100° C.). The PAOs are typically comprised of relatively low molecular weight hydrogenated polymers or oligomers of alphaolefins which include, but are not limited to, C<sub>2</sub> to about C<sub>32</sub> alphaolefins with the C<sub>8</sub> to about C<sub>16</sub> alphaolefins, such as 1-octene, 1-decene, 1-dodecene and the like, being preferred. The preferred polyalphaolefins are poly-1-octene, poly-1-decene and poly-1-dodecene and mixtures thereof and mixed olefin-derived polyolefins. However, the dimers of higher olefins in the range of C<sub>12</sub> to C<sub>18</sub> may be used to provide low viscosity base stocks of acceptably low volatility. Depending on the viscosity grade and the starting oligomer, the PAOs may be predominantly dimers, trimers and tetramers of the starting olefins, with minor amounts of the lower and/or higher oligomers, having a viscosity range of 1.5 cSt to 12 cSt. PAO fluids of particular use may include 3 cSt, 3.4 cSt, and/or 3.6 cSt and combinations thereof. Mixtures of PAO fluids having a viscosity range of 1.5 cSt to approximately 150 cSt or more may be used if desired. Unless indicated otherwise, all viscosities cited herein are measured at 100° C.

The PAO fluids may be conveniently made by the polymerization of an alphaolefin in the presence of a polymerization catalyst such as the Friedel-Crafts catalysts including, for example, aluminum trichloride, boron trifluoride or complexes of boron trifluoride with water, alcohols such as ethanol, propanol or butanol, carboxylic acids or esters such as ethyl acetate or ethyl propionate. For example the methods disclosed by U.S. Pat. No. 4,149,178 or 3,382,291 may be conveniently used herein. Other descriptions of PAO synthesis are found in the following U.S. Pat. Nos. 3,742,082; 3,769,363; 3,876,720; 4,239,930; 4,367,352; 4,413,156; 4,434,408; 4,910,355; 4,956,122; and 5,068,487. The dimers of the C<sub>14</sub> to C<sub>18</sub> olefins are described in U.S. Pat. No. 4,218,330.

Other useful lubricant oil base stocks include wax isomerate base stocks and base oils, comprising hydroisomerized waxy stocks (e.g. waxy stocks such as gas oils, slack waxes, fuels hydrocracker bottoms, etc.), hydroisomerized Fischer-Tropsch waxes, Gas-to-Liquids (GTL) base stocks and base oils, and other wax isomerate hydroisomerized base stocks and base oils, or mixtures thereof. Fischer-Tropsch waxes, the high boiling point residues of Fischer-Tropsch synthesis, are highly paraffinic hydrocarbons with very low sulfur content. The hydroprocessing used for the production of such base stocks may use an amorphous hydrocracking/hydroisomerization catalyst, such as one of the specialized lube hydrocracking (LHDC) catalysts or a crystalline hydrocracking/hydroisomerization catalyst, preferably a zeolitic catalyst. For example, one useful catalyst is ZSM-48 as described in U.S. Pat. No. 5,075,269, the disclosure of which is incorporated herein by reference in its entirety. Processes for making hydrocracked/hydroisomerized distillates and hydrocracked/hydroisomerized waxes are described, for example, in U.S. Pat. Nos. 2,817,693; 4,975,177; 4,921,594 and 4,897,178 as well as in British Patent Nos. 1,429,494; 1,350,257; 1,440,230 and 1,390,359. Each of the aforementioned patents is incorporated herein in their entirety. Particularly favorable processes are described in European

Patent Application Nos. 464546 and 464547, also incorporated herein by reference. Processes using Fischer-Tropsch wax feeds are described in U.S. Pat. Nos. 4,594,172 and 4,943,672, the disclosures of which are incorporated herein by reference in their entirety.

Gas-to-Liquids (GTL) base oils, Fischer-Tropsch wax derived base oils, and other wax-derived hydroisomerized (wax isomerate) base oils be advantageously used in the instant disclosure, and may have useful kinematic viscosities 10 at 100° C. of about 2 cSt to about 50 cSt, preferably about 2 cSt to about 30 cSt, more preferably about 3 cSt to about 25 cSt, as exemplified by GTL 4 with kinematic viscosity of about 4.0 cSt at 100° C. and a viscosity index of about 141. These Gas-to-Liquids (GTL) base oils, Fischer-Tropsch wax 15 derived base oils, and other wax-derived hydroisomerized base oils may have useful pour points of about -20° C. or lower, and under some conditions may have advantageous pour points of about -25° C. or lower, with useful pour points of about -30° C. to about -40° C. or lower. Useful 20 compositions of Gas-to-Liquids (GTL) base oils, Fischer-Tropsch wax derived base oils, and wax-derived hydroisomerized base oils are recited in U.S. Pat. Nos. 6,080,301; 6,090,989, and 6,165,949 for example, and are incorporated herein in their entirety by reference.

The hydrocarbyl aromatics can be used as a base oil or base oil component and can be any hydrocarbyl molecule that contains at least about 5% of its weight derived from an aromatic moiety such as a benzenoid moiety or naphthenoid moiety, or their derivatives. These hydrocarbyl aromatics 30 include alkyl benzenes, alkyl naphthalenes, alkyl biphenyls, alkyl diphenyl oxides, alkyl naphthols, alkyl diphenyl sulfides, alkylated bis-phenol A, alkylated thiadiphenol, and the like. The aromatic can be mono-alkylated, dialkylated, poly-alkylated, and the like. The aromatic can be mono- or 35 poly-functionalized. The hydrocarbyl groups can also be comprised of mixtures of alkyl groups, alkenyl groups, alkynyl, cycloalkyl groups, cycloalkenyl groups and other related hydrocarbyl groups. The hydrocarbyl groups can range from about C<sub>6</sub> up to about C<sub>60</sub> with a range of about 40 C<sub>8</sub> to about C<sub>20</sub> often being preferred. A mixture of hydrocarbyl groups is often preferred, and up to about three such substituents may be present. The hydrocarbyl group can optionally contain sulfur, oxygen, and/or nitrogen containing substituents. The aromatic group can also be derived 45 from natural (petroleum) sources, provided at least about 5% of the molecule is comprised of an above-type aromatic moiety. Viscosities at 100° C. of approximately 2 cSt to about 50 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 926

Friedel-Crafts alkylation of aromatic compounds. See Friedel-Crafts and Related Reactions, Olah, G. A. (ed.), Interscience Publishers, New York, 1963. For example, an aromatic compound, such as benzene or naphthalene, is alkylated by an olefin, alkyl halide or alcohol in the presence of a Friedel-Crafts catalyst. See Friedel-Crafts and Related Reactions, Vol. 2, part 1, chapters 14, 17, and 18, See Olah, G. A. (ed.), Interscience Publishers, New York, 1964. Many homogeneous or heterogeneous, solid catalysts are known to one skilled in the art. The choice of catalyst depends on the reactivity of the starting materials and product quality requirements. For example, strong acids such as  $\text{AlCl}_3$ ,  $\text{BF}_3$ , or HF may be used. In some cases, milder catalysts such as  $\text{FeCl}_3$  or  $\text{SnCl}_4$  are preferred. Newer alkylation technology uses zeolites or solid super acids.

Esters comprise a useful base stock. Additive solvency and seal compatibility characteristics may be secured by the use of esters such as the esters of dibasic acids with monoalkanols and the polyol esters of monocarboxylic acids. Esters of the former type include, for example, the esters of dicarboxylic acids such as phthalic acid, succinic acid, alkyl succinic acid, alkanyl succinic acid, maleic acid, azelaic acid, suberic acid, sebatic acid, fumaric acid, adipic acid, linoleic acid dimer, malonic acid, alkyl malonic acid, alkanyl malonic acid, etc., with a variety of alcohols such as butyl alcohol, hexyl alcohol, dodecyl alcohol, 2-ethylhexyl alcohol, etc. Specific examples of these types of esters include dibutyl adipate, di(2-ethylhexyl) sebacate, di-n-hexyl fumarate, dioctyl sebacate, diisooctyl azelate, diisodecyl azelate, dioctyl phthalate, didecyl phthalate, dieicosyl sebacate, etc.

Particularly useful synthetic esters are those which are obtained by reacting one or more polyhydric alcohols, preferably the hindered polyols (such as the neopentyl polyols, e.g., neopentyl glycol, trimethylol ethane, 2-methyl-2-propyl-1,3-propanediol, trimethylol propane, pentaerythritol and dipentaerythritol) with alkanoic acids containing at least about 4 carbon atoms, preferably  $\text{C}_5$  to  $\text{C}_{30}$  acids such as saturated straight chain fatty acids including caprylic acid, capric acid, lauric acid, myristic acid, palmitic acid, stearic acid, arachic acid, and behenic acid, or the corresponding branched chain fatty acids or unsaturated fatty acids such as oleic acid, or mixtures of any of these materials.

Suitable synthetic ester components include the esters of trimethylol propane, trimethylol butane, trimethylol ethane, pentaerythritol and/or dipentaerythritol with one or more monocarboxylic acids containing from about 5 to about 10 carbon atoms. These esters are widely available commercially, for example, the Mobil P-41 and P-51 esters of ExxonMobil Chemical Company.

Also useful are esters derived from renewable material such as coconut, palm, rapeseed, soy, sunflower and the like. These esters may be monoesters, di-esters, polyol esters, complex esters, or mixtures thereof. These esters are widely available commercially, for example, the Mobil P-51 ester of ExxonMobil Chemical Company.

Engine oil formulations containing renewable esters are included in this disclosure. For such formulations, the renewable content of the ester is typically greater than about 70 weight percent, preferably more than about 80 weight percent and most preferably more than about 90 weight percent.

Other useful fluids of lubricating viscosity include non-conventional or unconventional base stocks that have been processed, preferably catalytically, or synthesized to provide high performance lubrication characteristics.

Non-conventional or unconventional base stocks/base oils include one or more of a mixture of base stock(s) derived from one or more Gas-to-Liquids (GTL) materials, as well as isomerate/isodewaxate base stock(s) derived from natural wax or waxy feeds, mineral and or non-mineral oil waxy feed stocks such as slack waxes, natural waxes, and waxy stocks such as gas oils, waxy fuels hydrocracker bottoms, waxy raffinate, hydrocrackate, thermal crackates, or other mineral, mineral oil, or even non-petroleum oil derived waxy materials such as waxy materials received from coal liquefaction or shale oil, and mixtures of such base stocks.

GTL materials are materials that are derived via one or more synthesis, combination, transformation, rearrangement, and/or degradation/deconstructive processes from gaseous carbon-containing compounds, hydrogen-containing compounds and/or elements as feed stocks such as hydrogen, carbon dioxide, carbon monoxide, water, methane, ethane, ethylene, acetylene, propane, propylene, propyne, butane, butylenes, and butynes. GTL base stocks and/or base oils are GTL materials of lubricating viscosity that are generally derived from hydrocarbons; for example, waxy synthesized hydrocarbons, that are themselves derived from simpler gaseous carbon-containing compounds, hydrogen-containing compounds and/or elements as feed stocks. GTL base stock(s) and/or base oil(s) include oils boiling in the lube oil boiling range (1) separated/fractionated from synthesized GTL materials such as, for example, by distillation and subsequently subjected to a final wax processing step which involves either or both of a catalytic dewaxing process, or a solvent dewaxing process, to produce lube oils of reduced/low pour point; (2) synthesized wax isomerates, comprising, for example, hydrodewaxed or hydroisomerized cat and/or solvent dewaxed synthesized wax or waxy hydrocarbons; (3) hydrodewaxed or hydroisomerized cat and/or solvent dewaxed Fischer-Tropsch (F-T) material (i.e., hydrocarbons, waxy hydrocarbons, waxes and possible analogous oxygenates); preferably hydrodewaxed or hydroisomerized/followed by cat and/or solvent dewaxing dewaxed F-T waxy hydrocarbons, or hydrodewaxed or hydroisomerized/followed by cat (or solvent) dewaxing dewaxed, F-T waxes, or mixtures thereof.

GTL base stock(s) and/or base oil(s) derived from GTL materials, especially, hydrodewaxed or hydroisomerized/ followed by cat and/or solvent dewaxed wax or waxy feed, preferably F-T material derived base stock(s) and/or base oil(s), are characterized typically as having kinematic viscosities at 100° C. of from about 2  $\text{mm}^2/\text{s}$  to about 50  $\text{mm}^2/\text{s}$  (ASTM D445). They are further characterized typically as having pour points of -5° C. to about -40° C. or lower (ASTM D97). They are also characterized typically as having viscosity indices of about 80 to about 140 or greater (ASTM D2270).

In addition, the GTL base stock(s) and/or base oil(s) are typically highly paraffinic (>90% saturates), and may contain mixtures of monocycloparaffins and multicycloparaffins in combination with non-cyclic isoparaffins. The ratio of the naphthenic (i.e., cycloparaffin) content in such combinations varies with the catalyst and temperature used. Further, GTL base stock(s) and/or base oil(s) typically have very low sulfur and nitrogen content, generally containing less than about 10 ppm, and more typically less than about 5 ppm of each of these elements. The sulfur and nitrogen content of GTL base stock(s) and/or base oil(s) obtained from F-T material, especially F-T wax, is essentially nil. In addition, the absence of phosphorus and aromatics make this materially especially suitable for the formulation of low SAP products.

The term GTL base stock and/or base oil and/or wax isomerate base stock and/or base oil is to be understood as embracing individual fractions of such materials of wide viscosity range as recovered in the production process, mixtures of two or more of such fractions, as well as mixtures of one or two or more low viscosity fractions with one, two or more higher viscosity fractions to produce a blend wherein the blend exhibits a target kinematic viscosity.

The GTL material, from which the GTL base stock(s) and/or base oil(s) is/are derived is preferably an F-T material (i.e., hydrocarbons, waxy hydrocarbons, wax).

Base oils for use in the formulated lubricating oils useful in the present disclosure are any of the variety of oils corresponding to API Group I, Group II, Group III, Group IV, and Group V oils and mixtures thereof, preferably API Group II, Group III, Group IV, and Group V oils and mixtures thereof, more preferably the Group III to Group V base oils due to their exceptional volatility, stability, viscometric and cleanliness features. Minor quantities of Group I stock, such as the amount used to dilute additives for blending into formulated lube oil products, can be tolerated but should be kept to a minimum, i.e. amounts only associated with their use as diluent/carrier oil for additives used on an "as-received" basis. Even in regard to the Group II stocks, it is preferred that the Group II stock be in the higher quality range associated with that stock, i.e. a Group II stock having a viscosity index in the range 100<VI<120.

The base oil constitutes the major component of the engine oil lubricant composition of the present disclosure and typically is present in an amount ranging from about 6 to about 99 weight percent or from about 6 to about 95 weight percent, preferably from about 50 to about 99 weight percent or from about 70 to about 95 weight percent, and more preferably from about 85 to about 95 weight percent, based on the total weight of the composition. The base oil may be selected from any of the synthetic or natural oils typically used as crankcase lubricating oils for spark-ignited and compression-ignited engines. The base oil conveniently has a kinematic viscosity, according to ASTM standards, of about 2.5 cSt to about 18 cSt (or mm<sup>2</sup>/s) at 100° C. and preferably of about 2.5 cSt to about 12.5 cSt (or mm<sup>2</sup>/s) at 100° C., often more preferably from about 2.5 cSt to about 10 cSt. Mixtures of synthetic and natural base oils may be used if desired. Bi-modal, tri-modal, and additional combinations of mixtures of Group I, II, III, IV, and/or V base stocks may be used if desired.

The co-base stock component is present in an amount sufficient for providing solubility, compatibility and dispersancy of polar additives in the lubricating oil. The co-base stock component is present in the lubricating oils of this disclosure in an amount from about 1 to about 99 weight percent, preferably from about 5 to about 95 weight percent, and more preferably from about 10 to about 90 weight percent.

#### Molybdenum-Containing Compounds

Illustrative molybdenum-containing compounds useful in the disclosure include, for example, an oil-soluble decomposable organo molybdenum compound, such as Molyvan™ 855 which is an oil soluble secondary diarylamine defined as substantially free of active phosphorus and active sulfur. The Molyvan™ 855 is described in Vanderbilt's Material Data and Safety Sheet as a organomolybdenum compound having a density of 1.04 and viscosity at 100° C. of 47.12 cSt. In general, organo molybdenum compounds are preferred because of their superior solubility and effectiveness.

Another illustrative molybdenum-containing compound is Molyvan™ L which is sulfonated oxymolybdenum dialkyldithiophosphate described in U.S. Pat. No. 5,055,174 hereby incorporated by reference.

5 Molyvan™ A made by R. T. Vanderbilt Company, Inc., New York, N.Y., USA, is also an illustrative molybdenum-containing compound which contains about 28.8 wt. % Mo, 31.6 wt. % C, 5.4 wt. % H, and 25.9 wt. % S. Also useful are Molyvan™ 855, Molyvan™ 822, Molyvan™ 856, and Molyvan™ 807.

10 Also useful is Sakura Lube™ 500, which is more soluble Mo dithiocarbamate containing lubricant additive obtained from Asahi Denki Corporation and comprised of about 20.2 wt. % Mo, 43.8 wt. % C, 7.4 wt. % H, and 22.4 wt. % S.

15 Sakura Lube™ 300, a low sulfur molybdenum dithiophosphate having a molybdenum to sulfur ratio of 1:1.07, is a preferred molybdenum-containing compound useful in this disclosure.

Also useful is Molyvan™ 807, a mixture of about 50 wt. 20 % molybdenum ditridecylthiocarbonate, and about 50 wt. % of an aromatic oil having a specific gravity of about 38.4 SUS and containing about 4.6 wt. % molybdenum, also manufactured by R. T. Vanderbilt and marketed as an antioxidant and antiwear additive.

25 Other sources are molybdenum Mo(Co)<sub>6</sub>, and molybdenum octoate, MoO(C<sub>7</sub>H<sub>15</sub>CO<sub>2</sub>)<sub>2</sub> containing about 8 wt-% Mo marketed by Aldrich Chemical Company, Milwaukee, Wis. and molybdenum naphthenethiobisoctoate marketed by Shephard Chemical Company, Cincinnati, Ohio.

30 Inorganic molybdenum compounds such as molybdenum sulfide and molybdenum oxide are substantially less preferred than the organic compounds as described in Molyvan™ 855, Molyvan™ 822, Molyvan™ 856, and Molyvan™ 807.

35 Illustrative molybdenum-containing compounds useful in this disclosure are disclosed, for example, in U.S. Patent Application Publication No. 2003/0119682, which is incorporated herein by reference.

Whereas 1% is equal to 10,000 parts per million (ppm), 40 the preferred dosage in the molybdenum-containing compound is up to 5.0 percent by mass. More preferably the preferred dosage is up to 3,000 ppm by mass, more preferably from about 100 ppm to about 2,500 ppm by mass, more preferably from about 300 to about 2,000 ppm by mass, more preferably from 300 to about 1,500 ppm by mass of molybdenum.

#### Borated Ester Compounds

Illustrative boron-containing compounds useful in this disclosure include, for example, a borate ester, a boric acid, 50 other boron compounds such as a boron oxide. The boron compound is hydrolytically stable and is utilized for improved antiwear, and performs as a rust and corrosion inhibitor for copper bearings and other metal engine components. The borated ester compound acts as an inhibitor for 55 corrosion of metal to prevent corrosion of either ferrous or non-ferrous metals (e.g. copper, bronze, brass, titanium, aluminum and the like) or both, present in concentrations in which they are effective in inhibiting corrosion

Patents describing techniques for making basic salts of 60 sulfonic, carboxylic acids and mixtures thereof include U.S. Pat. Nos. 5,354,485; 2,501,731; 2,616,911; 2,777,874; 3,384,585; 3,320,162; 3,488,284; and 3,629,109. The disclosures of these patents are hereby incorporated by reference. Methods of preparing borated overbased compositions 65 are found in U.S. Pat. Nos. 4,744,920; 4,792,410; and PCT publication WO 88/03144. The disclosures of these references are hereby incorporated by reference. The oil-soluble

15

neutral or basic salts of alkali or alkaline earth metals salts may also be reacted with a boron compound.

An illustrative borate ester utilized in this disclosure is manufactured by Exxon-Mobil USA under the product designation of ("MCP 1286") and MOBIL ADC700. Test data show the viscosity at 100° C. using the D-445 method is 2.9 cSt; the viscosity at 40° C. using the D-445 method is 11.9; the flash point using the D-93 method is 146; the pour point using the D-97 method is -69; and the percent boron as determined by the ICP method is 5.3%. The borated ester (Vanlube<sup>TM</sup> 289), which is marketed as an antiwear/antscuff additive and friction reducer, is a preferred borate ester useful in this disclosure.

An illustrative borate ester useful in this disclosure is the reaction product obtained by reacting about 1 mole fatty oil, about 1.0 to 2.5 moles diethanolamine followed by subsequent reaction with boric acid to yield about 0.1 to 3 percent boron by mass. It is believed that the reaction products may include one or both of the following two primary components, with the further listed components being possible components when the reaction is pushed to toward full hydration:



where  $R_1 = H$  or  $C_xH_y$ , where  $x=1$  to 60, and  $y=3$  to 121



16

-continued



wherein Y represents a fatty oil residue. The preferred fatty oils are glycerol esters of higher fatty acids containing at least 12 carbon atoms and may contain 22 carbon atoms and higher. Such esters are commonly known as vegetable and animal oils. Vegetable oils particularly useful are oils derived from coconut, corn, cottonseed, linseed, peanut, soybean and sunflower seed. Similarly, animal fatty oils such as tallow may be used.

The source of boron is boric acid or materials that afford boron and are capable of reacting with the intermediate reaction product of fatty oil and diethanolamine to form a borate ester composition.

While the above organoborate ester composition is specifically discussed above, it should be understood that other organoborate ester compositions should also function with similar effect in the present disclosure, such as those set forth in U.S. Patent Application Publication No. 2003/0119682, which is incorporated herein by reference. In addition, dispersions of borate salts, such as potassium borate, may also be useful.

Other illustrative organoborate compositions useful in this disclosure are disclosed, for example, in U.S. Patent Application Publication No. 2008/0261838, which is incorporated herein by reference.

In addition, other illustrative organoborate compositions useful in this disclosure are disclosed, for example, U.S. Pat. No. 4,478,732, U.S. Pat. No. 4,406,802, U.S. Pat. No. 4,568,472 on borated mixed hydroxyl esters, alkoxylated amides, and amines; U.S. Pat. No. 4,298,486 on borated hydroxyethyl imidazolines; U.S. Pat. No. 4,328,113 on borated alkyl amines and alkyl diamines; U.S. Pat. No. 4,370,248 on borated hydroxyl-containing esters, including GMO; U.S. Pat. No. 4,374,032 on borated hydroxyl-containing hydrocarbyl oxazolines; U.S. Pat. No. 4,376,712 on borated sorbitan esters; U.S. Pat. No. 4,382,006 on borated ethoxylated amines; U.S. Pat. No. 4,389,322 on ethoxylated amides and their borates; U.S. Pat. No. 4,472,289 on hydrocarbyl vicinal diols and alcohols and ester mixtures and their borates; U.S. Pat. No. 4,522,734 on borates of hydrolyzed hydrocarbyl epoxides; U.S. Pat. No. 4,537,692 on ether-diamine borates; U.S. Pat. No. 4,541,941 on mixtures containing vicinal diols and hydroxyl substituted esters and their borates; U.S. Pat. No. 4,594,171 on borated mixtures of various hydroxyl and/or nitrogen containing borates; and

U.S. Pat. No. 4,692,257 on various borated alcohols/diols, which are incorporated herein by reference.

The preferred dosage of boron compound in the total lubricant is up to 10.0 volume percent, more preferably from about 0.01 to about 10.0 volume %, more preferably from about 0.01 to about 5 volume %, and most preferably from about 0.1-3.0 volume %. An effective elemental boron range of up to 1000 ppm or less than 1% elemental boron. Thus, a preferred concentration of elemental boron is from 100 to 1000 ppm and more preferably from 100 to 300 ppm.

#### Other Additives

The formulated lubricating oil useful in the present disclosure may additionally contain one or more of the other commonly used lubricating oil performance additives including but not limited to antiwear additives, dispersants, detergents, viscosity modifiers, corrosion inhibitors, rust inhibitors, metal deactivators, extreme pressure additives, anti-seizure agents, wax modifiers, viscosity modifiers, fluid-loss additives, seal compatibility agents, lubricity agents, anti-staining agents, chromophoric agents, defoamants, demulsifiers, densifiers, wetting agents, gelling agents, tackiness agents, colorants, and others. For a review of many commonly used additives, see Klamann in Lubricants and Related Products, Verlag Chemie, Deerfield Beach, Fla.; ISBN 0-89573-177-0. Reference is also made to "Lubricant Additives" by M. W. Ranney, published by Noyes Data Corporation of Parkridge, N J (1973); see also U.S. Pat. No. 7,704,930, the disclosure of which is incorporated herein in its entirety. These additives are commonly delivered with varying amounts of diluent oil, that may range from 5 weight percent to 50 weight percent.

The additives useful in this disclosure do not have to be soluble in the lubricating oils. Insoluble additives in oil can be dispersed in the lubricating oils of this disclosure.

The types and quantities of performance additives used in combination with the instant disclosure in lubricant compositions are not limited by the examples shown herein as illustrations.

#### Antiwear Additives

A metal alkylthiophosphate and more particularly a metal dialkyl dithio phosphate in which the metal constituent is zinc, or zinc dialkyl dithio phosphate (ZDDP) can be a useful component of the lubricating oils of this disclosure. ZDDP can be derived from primary alcohols, secondary alcohols or mixtures thereof. ZDDP compounds generally are of the formula



where R<sup>1</sup> and R<sup>2</sup> are C<sub>1</sub>-C<sub>18</sub> alkyl groups, preferably C<sub>2</sub>-C<sub>12</sub> alkyl groups. These alkyl groups may be straight chain or branched. Alcohols used in the ZDDP can be propanol, 2-propanol, butanol, secondary butanol, pentanols, hexanols such as 4-methyl-2-pentanol, n-hexanol, n-octanol, 2-ethyl hexanol, alkylated phenols, and the like. Mixtures of secondary alcohols or of primary and secondary alcohol can be preferred. Alkyl aryl groups may also be used.

Preferable zinc dithiophosphates which are commercially available include secondary zinc dithiophosphates such as those available from for example, The Lubrizol Corporation under the trade designations "LZ 677A", "LZ 1095" and "LZ 1371", from for example Chevron Oronite under the trade designation "OLOA 262" and from for example Afton Chemical under the trade designation "HITEC 7169".

The ZDDP is typically used in amounts of from about 0.3 weight percent to about 1.5 weight percent, preferably from about 0.4 weight percent to about 1.2 weight percent, more preferably from about 0.5 weight percent to about 1.0 weight

percent, and even more preferably from about 0.6 weight percent to about 0.8 weight percent, based on the total weight of the lubricating oil, although more or less can often be used advantageously. Preferably, the ZDDP is a secondary ZDDP and present in an amount of from about 0.6 to 1.0 weight percent of the total weight of the lubricating oil. Dispersants

During engine operation, oil-insoluble oxidation byproducts are produced. Dispersants help keep these byproducts in solution, thus diminishing their deposition on metal surfaces. Dispersants used in the formulation of the lubricating oil may be ashless or ash-forming in nature. Preferably, the dispersant is ashless. So called ashless dispersants are organic materials that form substantially no ash upon combustion. For example, non-metal-containing or borated metal-free dispersants are considered ashless. In contrast, metal-containing detergents discussed above form ash upon combustion.

Suitable dispersants typically contain a polar group attached to a relatively high molecular weight hydrocarbon chain. The polar group typically contains at least one element of nitrogen, oxygen, or phosphorus. Typical hydrocarbon chains contain 50 to 400 carbon atoms.

A particularly useful class of dispersants are the (poly) alkenylsuccinic derivatives, typically produced by the reaction of a long chain hydrocarbyl substituted succinic compound, usually a hydrocarbyl substituted succinic anhydride, with a polyhydroxy or polyamino compound. The long chain hydrocarbyl group constituting the oleophilic portion of the molecule which confers solubility in the oil, is normally a polyisobutylene group. Many examples of this type of dispersant are well known commercially and in the literature. Exemplary U.S. patents describing such dispersants are U.S. Pat. Nos. 3,172,892; 3,2145,707; 3,219,666; 3,316,177; 3,341,542; 3,444,170; 3,454,607; 3,541,012; 3,630,904; 3,632,511; 3,787,374 and 4,234,435. Other types of dispersant are described in U.S. Pat. Nos. 3,036,003; 3,200,107; 3,254,025; 3,275,554; 3,438,757; 3,454,555; 3,565,804; 3,413,347; 3,697,574; 3,725,277; 3,725,480; 3,726,882; 4,454,059; 3,329,658; 3,449,250; 3,519,565; 3,666,730; 3,687,849; 3,702,300; 4,100,082; 5,705,458. A further description of dispersants may be found, for example, in European Patent Application No. 471 071, to which reference is made for this purpose.

Hydrocarbyl-substituted succinic acid and hydrocarbyl-substituted succinic anhydride derivatives are useful dispersants. In particular, succinimide, succinate esters, or succinate ester amides prepared by the reaction of a hydrocarbon-substituted succinic acid compound preferably having at least 50 carbon atoms in the hydrocarbon substituent, with at least one equivalent of an alkylene amine are particularly useful.

Succinimides are formed by the condensation reaction between hydrocarbyl substituted succinic anhydrides and amines. Molar ratios can vary depending on the polyamine. For example, the molar ratio of hydrocarbyl substituted succinic anhydride to TEPA can vary from about 1:1 to about 5:1. Representative examples are shown in U.S. Pat. Nos. 3,087,936; 3,172,892; 3,219,666; 3,272,746; 3,322,670; and U.S. Pat. Nos. 3,652,616, 3,948,800; and Canada Patent No. 1,094,044.

Succinate esters are formed by the condensation reaction between hydrocarbyl substituted succinic anhydrides and alcohols or polyols. Molar ratios can vary depending on the alcohol or polyol used. For example, the condensation product of a hydrocarbyl substituted succinic anhydride and pentaerythritol is a useful dispersant.

Succinate ester amides are formed by condensation reaction between hydrocarbyl substituted succinic anhydrides and alkanol amines. For example, suitable alkanol amines include ethoxylated polyalkylpolyamines, propoxylated polyalkylpolyamines and polyalkenylpolyamines such as polyethylene polyamines. One example is propoxylated hexamethylenediamine. Representative examples are shown in U.S. Pat. No. 4,426,305.

The molecular weight of the hydrocarbyl substituted succinic anhydrides used in the preceding paragraphs will typically range between 800 and 2,500 or more. The above products can be post-reacted with various reagents such as sulfur, oxygen, formaldehyde, carboxylic acids such as oleic acid. The above products can also be post reacted with boron compounds such as boric acid, borate esters or highly borated dispersants, to form borated dispersants generally having from about 0.1 to about 5 moles of boron per mole of dispersant reaction product.

Mannich base dispersants are made from the reaction of alkylphenols, formaldehyde, and amines. See U.S. Pat. No. 4,767,551, which is incorporated herein by reference. Process aids and catalysts, such as oleic acid and sulfonic acids, can also be part of the reaction mixture. Molecular weights of the alkylphenols range from 800 to 2,500. Representative examples are shown in U.S. Pat. Nos. 3,697,574; 3,703,536; 3,704,308; 3,751,365; 3,756,953; 3,798,165; and 3,803,039.

Typical high molecular weight aliphatic acid modified Mannich condensation products useful in this disclosure can be prepared from high molecular weight alkyl-substituted hydroxyaromatics or HNR<sub>2</sub> group-containing reactants.

Hydrocarbyl substituted amine ashless dispersant additives are well known to one skilled in the art; see, for example, U.S. Pat. Nos. 3,275,554; 3,438,757; 3,565,804; 3,755,433, 3,822,209, and 5,084,197.

Preferred dispersants include borated and non-borated succinimides, including those derivatives from mono-succinimides, bis-succinimides, and/or mixtures of mono- and bis-succinimides, wherein the hydrocarbyl succinimide is derived from a hydrocarbylene group such as polyisobutylene having a Mn of from about 500 to about 5000, or from about 1000 to about 3000, or about 1000 to about 2000, or a mixture of such hydrocarbylene groups, often with high terminal vinylidene groups. Other preferred dispersants include succinic acid-esters and amides, alkylphenol-polyamine-coupled Mannich adducts, their capped derivatives, and other related components.

Polymethacrylate or polyacrylate derivatives are another class of dispersants. These dispersants are typically prepared by reacting a nitrogen containing monomer and a methacrylic or acrylic acid esters containing 5-25 carbon atoms in the ester group. Representative examples are shown in U.S. Pat. Nos. 2,100,993, and 6,323,164. Polymethacrylate and polyacrylate dispersants are normally used as multifunctional viscosity modifiers. The lower molecular weight versions can be used as lubricant dispersants or fuel detergents.

Illustrative preferred dispersants useful in this disclosure include those derived from polyalkenyl-substituted mono- or dicarboxylic acid, anhydride or ester, which dispersant has a polyalkenyl moiety with a number average molecular weight of at least 900 and from greater than 1.3 to 1.7, preferably from greater than 1.3 to 1.6, most preferably from greater than 1.3 to 1.5, functional groups (mono- or dicarboxylic acid producing moieties) per polyalkenyl moiety (a medium functionality dispersant). Functionality (F) can be determined according to the following formula:

$$F = (SAP \times M_n) / ((112,200 \times A.I.) - (SAP \times 98))$$

wherein SAP is the saponification number (i.e., the number of milligrams of KOH consumed in the complete neutralization of the acid groups in one gram of the succinic-containing reaction product, as determined according to ASTM D94); M<sub>n</sub> is the number average molecular weight of the starting olefin polymer; and A.I. is the percent active ingredient of the succinic-containing reaction product (the remainder being unreacted olefin polymer, succinic anhydride and diluent).

The polyalkenyl moiety of the dispersant may have a number average molecular weight of at least 900, suitably at least 1500, preferably between 1800 and 3000, such as between 2000 and 2800, more preferably from about 2100 to 2500, and most preferably from about 2200 to about 2400. The molecular weight of a dispersant is generally expressed in terms of the molecular weight of the polyalkenyl moiety. This is because the precise molecular weight range of the dispersant depends on numerous parameters including the type of polymer used to derive the dispersant, the number of functional groups, and the type of nucleophilic group employed.

Polymer molecular weight, specifically M<sub>n</sub>, can be determined by various known techniques. One convenient method is gel permeation chromatography (GPC), which additionally provides molecular weight distribution information (see W. W. Yau, J. J. Kirkland and D. D. Bly, "Modern Size Exclusion Liquid Chromatography", John Wiley and Sons, New York, 1979). Another useful method for determining molecular weight, particularly for lower molecular weight polymers, is vapor pressure osmometry (e.g., ASTM D3592).

The polyalkenyl moiety in a dispersant preferably has a narrow molecular weight distribution (MWD), also referred to as polydispersity, as determined by the ratio of weight average molecular weight (M<sub>w</sub>) to number average molecular weight (M<sub>n</sub>). Polymers having a M<sub>w</sub>/M<sub>n</sub> of less than 2.2, preferably less than 2.0, are most desirable. Suitable polymers have a polydispersity of from about 1.5 to 2.1, preferably from about 1.6 to about 1.8.

Suitable polyalkenes employed in the formation of the dispersants include homopolymers, interpolymers or lower molecular weight hydrocarbons. One family of such polymers comprise polymers of ethylene and/or at least one C<sub>3</sub> to C<sub>2</sub> alpha-olefin having the formula H<sub>2</sub>C=CHR<sup>1</sup> wherein R<sup>1</sup> is a straight or branched chain alkyl radical comprising 1 to 26 carbon atoms and wherein the polymer contains carbon-to-carbon unsaturation, and a high degree of terminal ethenylidene unsaturation. Preferably, such polymers comprise interpolymers of ethylene and at least one alpha-olefin of the above formula, wherein R<sup>1</sup> is alkyl of from 1 to 18 carbon atoms, and more preferably is alkyl of from 1 to 8 carbon atoms, and more preferably still of from 1 to 2 carbon atoms.

Another useful class of polymers is polymers prepared by cationic polymerization of monomers such as isobutene and styrene. Common polymers from this class include polyisobutenes obtained by polymerization of a C<sub>4</sub> refinery stream having a butene content of 35 to 75% by wt., and an isobutene content of 30 to 60% by wt. A preferred source of monomer for making poly-n-butenes is petroleum feedstreams such as Raffinate II. These feedstocks are disclosed in the art such as in U.S. Pat. No. 4,952,739. A preferred embodiment utilizes polyisobutylene prepared from a pure isobutylene stream or a Raffinate I stream to prepare reactive isobutylene polymers with terminal vinylidene olefins. Polyisobutene polymers that may be employed are generally based on a polymer chain of from 1500 to 3000.

The dispersant(s) are preferably non-polymeric (e.g., mono- or bis-succinimides). Such dispersants can be prepared by conventional processes such as disclosed in U.S. Patent Application Publication No. 2008/0020950, the disclosure of which is incorporated herein by reference.

The dispersant(s) can be borated by conventional means, as generally disclosed in U.S. Pat. Nos. 3,087,936, 3,254,025 and 5,430,105.

Such dispersants may be used in an amount of about 0.01 to 20 weight percent or 0.01 to 10 weight percent, preferably about 0.5 to 8 weight percent, or more preferably 0.5 to 4 weight percent. Or such dispersants may be used in an amount of about 2 to 12 weight percent, preferably about 4 to 10 weight percent, or more preferably 6 to 9 weight percent. On an active ingredient basis, such additives may be used in an amount of about 0.06 to 14 weight percent, preferably about 0.3 to 6 weight percent. The hydrocarbon portion of the dispersant atoms can range from C<sub>60</sub> to C<sub>1000</sub>, or from C<sub>70</sub> to C<sub>300</sub>, or from C<sub>70</sub> to C<sub>200</sub>. These dispersants may contain both neutral and basic nitrogen, and mixtures of both. Dispersants can be end-capped by borates and/or cyclic carbonates. Nitrogen content in the finished oil can vary from about 200 ppm by weight to about 2000 ppm by weight, preferably from about 200 ppm by weight to about 1200 ppm by weight. Basic nitrogen can vary from about 100 ppm by weight to about 1000 ppm by weight, preferably from about 100 ppm by weight to about 600 ppm by weight.

Dispersants as described herein are beneficially useful with the compositions of this disclosure and substitute for some or all of the surfactants of this disclosure. Further, in one embodiment, preparation of the compositions of this disclosure using one or more dispersants is achieved by combining ingredients of this disclosure, plus optional base stocks and lubricant additives, in a mixture at a temperature above the melting point of such ingredients, particularly that of the one or more M-carboxylates (M=H, metal, two or more metals, mixtures thereof).

As used herein, the dispersant concentrations are given on an "as delivered" basis. Typically, the active dispersant is delivered with a process oil. The "as delivered" dispersant typically contains from about 20 weight percent to about 80 weight percent, or from about 40 weight percent to about 60 weight percent, of active dispersant in the "as delivered" dispersant product.

#### Detergents

Illustrative detergents useful in this disclosure include, for example, alkali metal detergents, alkaline earth metal detergents, or mixtures of one or more alkali metal detergents and one or more alkaline earth metal detergents. A typical detergent is an anionic material that contains a long chain hydrophobic portion of the molecule and a smaller anionic or oleophobic hydrophilic portion of the molecule. The anionic portion of the detergent is typically derived from an organic acid such as a sulfur-containing acid, carboxylic acid (e.g., salicylic acid), phosphorus-containing acid, phenol, or mixtures thereof. The counterion is typically an alkaline earth or alkali metal. The detergent can be overbased as described herein.

The detergent is preferably a metal salt of an organic or inorganic acid, a metal salt of a phenol, or mixtures thereof. The metal is preferably selected from an alkali metal, an alkaline earth metal, and mixtures thereof. The organic or inorganic acid is selected from an aliphatic organic or inorganic acid, a cycloaliphatic organic or inorganic acid, an aromatic organic or inorganic acid, and mixtures thereof.

The metal is preferably selected from an alkali metal, an alkaline earth metal, and mixtures thereof. More preferably, the metal is selected from calcium (Ca), magnesium (Mg), and mixtures thereof.

The organic acid or inorganic acid is preferably selected from a sulfur-containing acid, a carboxylic acid, a phosphorus-containing acid, and mixtures thereof.

Preferably, the metal salt of an organic or inorganic acid or the metal salt of a phenol comprises calcium phenate, calcium sulfonate, calcium salicylate, magnesium phenate, magnesium sulfonate, magnesium salicylate, an overbased detergent, and mixtures thereof.

Salts that contain a substantially stoichiometric amount of the metal are described as neutral salts and have a total base number (TBN, as measured by ASTM D2896) of from 0 to 80. Many compositions are overbased, containing large amounts of a metal base that is achieved by reacting an excess of a metal compound (a metal hydroxide or oxide, for example) with an acidic gas (such as carbon dioxide). Useful detergents can be neutral, mildly overbased, or highly overbased. These detergents can be used in mixtures of neutral, overbased, highly overbased calcium salicylate, sulfonates, phenates and/or magnesium salicylate, sulfonates, phenates. The TBN ranges can vary from low, medium to high TBN products, including as low as 0 to as high as 600. Preferably the TBN delivered by the detergent is between 1 and 20. More preferably between 1 and 12. Mixtures of low, medium, high TBN can be used, along with mixtures of calcium and magnesium metal based detergents, and including sulfonates, phenates, salicylates, and carboxylates. A detergent mixture with a metal ratio of 1, in conjunction of a detergent with a metal ratio of 2, and as high as a detergent with a metal ratio of 5, can be used. Borated detergents can also be used.

Alkaline earth phenates are another useful class of detergent. These detergents can be made by reacting alkaline earth metal hydroxide or oxide (CaO, Ca(OH)<sub>2</sub>, BaO, Ba(OH)<sub>2</sub>, MgO, Mg(OH)<sub>2</sub>, for example) with an alkyl phenol or sulfurized alkylphenol. Useful alkyl groups include straight chain or branched C<sub>1</sub>-C<sub>30</sub> alkyl groups, preferably, C<sub>4</sub>-C<sub>20</sub> or mixtures thereof. Examples of suitable phenols include isobutylphenol, 2-ethylhexylphenol, nonylphenol, dodecyl phenol, and the like. It should be noted that starting alkylphenols may contain more than one alkyl substituent that are each independently straight chain or branched and can be used from 0.5 to 6 weight percent. When a non-sulfurized alkylphenol is used, the sulfurized product may be obtained by methods well known in the art. These methods include heating a mixture of alkylphenol and sulfurizing agent (including elemental sulfur, sulfur halides such as sulfur dichloride, and the like) and then reacting the sulfurized phenol with an alkaline earth metal base.

In accordance with this disclosure, metal salts of carboxylic acids are preferred detergents. These carboxylic acid detergents may be prepared by reacting a basic metal compound with at least one carboxylic acid and removing free water from the reaction product. These compounds may be overbased to produce the desired TBN level. Detergents made from salicylic acid are one preferred class of detergents derived from carboxylic acids. Useful salicylates include long chain alkyl salicylates. One useful family of compositions is of the formula



where R is an alkyl group having 1 to about 30 carbon atoms, n is an integer from 1 to 4, and M is an alkaline earth metal. Preferred R groups are alkyl chains of at least C<sub>11</sub>, preferably C<sub>13</sub> or greater. R may be optionally substituted with substituents that do not interfere with the detergent's function. M is preferably, calcium, magnesium, barium, or mixtures thereof. More preferably, M is calcium.

Hydrocarbyl-substituted salicylic acids may be prepared from phenols by the Kolbe reaction (see U.S. Pat. No. 3,595,791). The metal salts of the hydrocarbyl-substituted salicylic acids may be prepared by double decomposition of a metal salt in a polar solvent such as water or alcohol.

Alkaline earth metal phosphates are also used as detergents and are known in the art.

Detergents may be simple detergents or what is known as hybrid or complex detergents. The latter detergents can provide the properties of two detergents without the need to blend separate materials. See U.S. Pat. No. 6,034,039.

Preferred detergents include calcium sulfonates, magnesium sulfonates, calcium salicylates, magnesium salicylates, calcium phenates, magnesium phenates, and other related components (including borated detergents), and mixtures thereof. Preferred mixtures of detergents include magnesium sulfonate and calcium salicylate, magnesium sulfonate and calcium sulfonate, magnesium sulfonate and calcium phenate, calcium phenate and calcium salicylate, calcium phenate and calcium sulfonate, calcium phenate and magnesium salicylate, calcium phenate and magnesium phenate. Overbased detergents are also preferred.

The detergent concentration in the lubricating oils of this disclosure can range from about 0.5 to about 6.0 weight percent, preferably about 0.6 to 5.0 weight percent, and more preferably from about 0.8 weight percent to about 4.0 weight percent, based on the total weight of the lubricating oil.

As used herein, the detergent concentrations are given on an "as delivered" basis. Typically, the active detergent is delivered with a process oil. The "as delivered" detergent typically contains from about 20 weight percent to about 100 weight percent, or from about 40 weight percent to about 60 weight percent, of active detergent in the "as delivered" detergent product.

#### Viscosity Modifiers

Viscosity modifiers (also known as viscosity index improvers (VI improvers), and viscosity improvers) can be included in the lubricant compositions of this disclosure.

Viscosity modifiers provide lubricants with high and low temperature operability. These additives impart shear stability at elevated temperatures and acceptable viscosity at low temperatures.

Suitable viscosity modifiers include high molecular weight hydrocarbons, polyesters and viscosity modifier dispersants that function as both a viscosity modifier and a dispersant. Typical molecular weights of these polymers are between about 10,000 to 1,500,000, more typically about 20,000 to 1,200,000, and even more typically between about 50,000 and 1,000,000.

Examples of suitable viscosity modifiers are linear or star-shaped polymers and copolymers of methacrylate, butadiene, olefins, or alkylated styrenes. Polyisobutylene is a commonly used viscosity modifier. Another suitable viscosity modifier is polymethacrylate (copolymers of various chain length alkyl methacrylates, for example), some formulations of which also serve as pour point depressants. Other suitable viscosity modifiers include copolymers of ethylene and propylene, hydrogenated block copolymers of styrene and isoprene, and polyacrylates (copolymers of various chain length acrylates, for example). Specific examples include styrene-isoprene or styrene-butadiene based polymers of 50,000 to 200,000 molecular weight.

Olefin copolymers are commercially available from 15 Chevron Oronite Company LLC under the trade designation "PARATONE®" (such as "PARATONE® 8921" and "PARATONE® 8941"); from Afton Chemical Corporation under the trade designation "HiTEC®" (such as "HiTEC® 5850B"); and from The Lubrizol Corporation under the trade 20 designation "Lubrizol® 7067C". Hydrogenated polyisoprene star polymers are commercially available from Infineum International Limited, e.g., under the trade designation "SV200" and "SV600". Hydrogenated diene-styrene block copolymers are commercially available from Infineum International Limited, e.g., under the trade designation "SV 50".

The polymethacrylate or polyacrylate polymers can be linear polymers which are available from Evonik Industries under the trade designation "Viscoplex®" (e.g., Viscoplex 30 6-954) or star polymers which are available from Lubrizol Corporation under the trade designation Asteric™ (e.g., Lubrizol 87708 and Lubrizol 87725).

Illustrative vinyl aromatic-containing polymers useful in this disclosure may be derived predominantly from vinyl aromatic hydrocarbon monomer. Illustrative vinyl aromatic-containing copolymers useful in this disclosure may be represented by the following general formula:



40 wherein A is a polymeric block derived predominantly from vinyl aromatic hydrocarbon monomer, and B is a polymeric block derived predominantly from conjugated diene monomer.

In an embodiment of this disclosure, the viscosity modifiers 45 may be used in an amount of less than about 10 weight percent, preferably less than about 7 weight percent, more preferably less than about 4 weight percent, and in certain instances, may be used at less than 2 weight percent, preferably less than about 1 weight percent, and more preferably less than about 0.5 weight percent, based on the total weight of the formulated oil or lubricating engine oil. Viscosity modifiers are typically added as concentrates, in large amounts of diluent oil.

As used herein, the viscosity modifier concentrations are 55 given on an "as delivered" basis. Typically, the active polymer is delivered with a diluent oil. The "as delivered" viscosity modifier typically contains from 20 weight percent to 75 weight percent of an active polymer for polymethacrylate or polyacrylate polymers, or from 8 weight percent to 20 weight percent of an active polymer for olefin copolymers, hydrogenated polyisoprene star polymers, or hydrogenated diene-styrene block copolymers, in the "as delivered" polymer concentrate.

#### Antioxidants

60 Antioxidants retard the oxidative degradation of base oils during service. Such degradation may result in deposits on metal surfaces, the presence of sludge, or a viscosity

increase in the lubricant. One skilled in the art knows a wide variety of oxidation inhibitors that are useful in lubricating oil compositions. See, Klamann in Lubricants and Related Products, op. cit., and U.S. Pat. Nos. 4,798,684 and 5,084,197, for example.

Useful antioxidants include hindered phenols. These phenolic antioxidants may be ashless (metal-free) phenolic compounds or neutral or basic metal salts of certain phenolic compounds. Typical phenolic antioxidant compounds are the hindered phenolics which are the ones which contain a sterically hindered hydroxyl group, and these include those derivatives of dihydroxy aryl compounds in which the hydroxyl groups are in the o- or p-position to each other. Typical phenolic antioxidants include the hindered phenols substituted with  $C_6+$  alkyl groups and the alkylene coupled derivatives of these hindered phenols. Examples of phenolic materials of this type 2-t-butyl-4-heptyl phenol; 2-t-butyl-4-octyl phenol; 2-t-butyl-4-dodecyl phenol; 2,6-di-t-butyl-4-heptyl phenol; 2,6-di-t-butyl-4-dodecyl phenol; 2-methyl-6-t-butyl-4-heptyl phenol; and 2-methyl-6-t-butyl-4-dodecyl phenol. Other useful hindered mono-phenolic antioxidants may include for example hindered 2,6-di-alkyl-phenolic propionic ester derivatives. Bis-phenolic antioxidants may also be advantageously used in combination with the instant disclosure. Examples of ortho-coupled phenols include: 2,2'-bis(4-heptyl-6-t-butyl-phenol); 2,2'-bis(4-octyl-6-t-butyl-phenol); and 2,2'-bis(4-dodecyl-6-t-butyl-phenol). Para-coupled bisphenols include for example 4,4'-bis(2,6-di-t-butyl phenol) and 4,4'-methylene-bis(2,6-di-t-butyl phenol).

Effective amounts of one or more catalytic antioxidants may also be used. The catalytic antioxidants comprise an effective amount of a) one or more oil soluble polymetal organic compounds; and, effective amounts of b) one or more substituted N,N'-diaryl-o-phenylenediamine compounds or c) one or more hindered phenol compounds; or a combination of both b) and c). Catalytic antioxidants are more fully described in U.S. Pat. No. 8,048,833, herein incorporated by reference in its entirety.

Non-phenolic oxidation inhibitors which may be used include aromatic amine antioxidants and these may be used either as such or in combination with phenolics. Typical examples of non-phenolic antioxidants include: alkylated and non-alkylated aromatic amines such as aromatic mono-amines of the formula  $R^8R^9R^{10}N$  where  $R^8$  is an aliphatic, aromatic or substituted aromatic group,  $R^9$  is an aromatic or a substituted aromatic group, and  $R^{10}$  is H, alkyl, aryl or  $R^{11}S(O)_xR^{12}$  where  $R^{11}$  is an alkylene, alkenylene, or aralkylene group,  $R^{12}$  is a higher alkyl group, or an alkenyl, aryl, or alkaryl group, and x is 0, 1 or 2. The aliphatic group  $R^8$  may contain from 1 to about 20 carbon atoms, and preferably contains from about 6 to 12 carbon atoms. The aliphatic group is a saturated aliphatic group. Preferably, both  $R^8$  and  $R^9$  are aromatic or substituted aromatic groups, and the aromatic group may be a fused ring aromatic group such as naphthyl. Aromatic groups  $R^8$  and  $R^9$  may be joined together with other groups such as S.

Typical aromatic amines antioxidants have alkyl substituent groups of at least about 6 carbon atoms. Examples of aliphatic groups include hexyl, heptyl, octyl, nonyl, and decyl. Generally, the aliphatic groups will not contain more than about 14 carbon atoms. The general types of amine antioxidants useful in the present compositions include diphenylamines, phenyl naphthylamines, phenothiazines, imidodibenzyls and diphenyl phenylene diamines. Mixtures of two or more aromatic amines are also useful. Polymeric amine antioxidants can also be used. Particular examples of aromatic amine antioxidants useful in the present disclosure

include: p,p'-dioctyldiphenylamine; t-octylphenyl-alpha-naphthylamine; phenyl-alpha-naphthylamine; and p-octylphenyl-alpha-naphthylamine.

Sulfurized alkyl phenols and alkali or alkaline earth metal salts thereof also are useful antioxidants.

Preferred antioxidants include hindered phenols, arylamines. These antioxidants may be used individually by type or in combination with one another. Such additives may be used in an amount of about 0.01 to 5 weight percent, preferably about 0.01 to 1.5 weight percent, more preferably zero to less than 1.5 weight percent, more preferably zero to less than 1 weight percent.

#### Pour Point Depressants (PPDs)

Conventional pour point depressants (also known as lube oil flow improvers) may be added to the compositions of the present disclosure if desired. These pour point depressant may be added to lubricating compositions of the present disclosure to lower the minimum temperature at which the fluid will flow or can be poured. Examples of suitable pour point depressants include polymethacrylates, polyacrylates, polyarylamides, condensation products of haloparaffin waxes and aromatic compounds, vinyl carboxylate polymers, and terpolymers of dialkylfumarates, vinyl esters of fatty acids and allyl vinyl ethers. U.S. Pat. Nos. 1,815,022; 2,015,748; 2,191,498; 2,387,501; 2,655, 479; 2,666,746; 2,721,877; 2,721,878; and 3,250,715 describe useful pour point depressants and/or the preparation thereof. Such additives may be used in an amount of about 0.01 to 5 weight percent, preferably about 0.01 to 1.5 weight percent.

#### Seal Compatibility Agents

Seal compatibility agents help to swell elastomeric seals by causing a chemical reaction in the fluid or physical change in the elastomer. Suitable seal compatibility agents for lubricating oils include organic phosphates, aromatic esters, aromatic hydrocarbons, esters (butylbenzyl phthalate, for example), and polybutenyl succinic anhydride. Such additives may be used in an amount of about 0.01 to 3 weight percent, preferably about 0.01 to 2 weight percent.

#### Antifoam Agents

Anti-foam agents may advantageously be added to lubricant compositions. These agents retard the formation of stable foams. Silicones and organic polymers are typical anti-foam agents. For example, polysiloxanes, such as silicon oil or polydimethyl siloxane, provide antifoam properties. Anti-foam agents are commercially available and may be used in conventional minor amounts along with other additives such as demulsifiers; usually the amount of these additives combined is less than 1 weight percent and often less than 0.1 weight percent.

#### Inhibitors and Antirust Additives

Antirust additives (or corrosion inhibitors) are additives that protect lubricated metal surfaces against chemical attack by water or other contaminants. A wide variety of these are commercially available.

One type of antirust additive is a polar compound that wets the metal surface preferentially, protecting it with a film of oil. Another type of antirust additive absorbs water by incorporating it in a water-in-oil emulsion so that only the oil touches the metal surface. Yet another type of antirust additive chemically adheres to the metal to produce a non-reactive surface. Examples of suitable additives include zinc dithiophosphates, metal phenolates, basic metal sulfonates, fatty acids and amines. Such additives may be used in an amount of about 0.01 to 5 weight percent, preferably about 0.01 to 1.5 weight percent.

## Friction Modifiers

A friction modifier is any material or materials that can alter the coefficient of friction of a surface lubricated by any lubricant or fluid containing such material(s). Friction modifiers, also known as friction reducers, or lubricity agents or oiliness agents, and other such agents that change the ability of base oils, formulated lubricant compositions, or functional fluids, to modify the coefficient of friction of a lubricated surface may be effectively used in combination with the base oils or lubricant compositions of the present disclosure if desired. Friction modifiers that lower the coefficient of friction are particularly advantageous in combination with the base oils and lube compositions of this disclosure.

Illustrative friction modifiers may include, for example, organometallic compounds or materials, or mixtures thereof. Illustrative organometallic friction modifiers useful in the lubricating engine oil formulations of this disclosure include, for example, molybdenum amine, molybdenum diamine, an organotungstenate, a molybdenum dithiocarbamate, molybdenum dithiophosphates, molybdenum amine complexes, molybdenum carboxylates, and the like, and mixtures thereof. Similar tungsten based compounds may be preferable.

Other illustrative friction modifiers useful in the lubricating engine oil formulations of this disclosure include, for example, alkoxylated fatty acid esters, alkanolamides, polyol fatty acid esters, borated glycerol fatty acid esters, fatty alcohol ethers, and mixtures thereof.

Illustrative alkoxylated fatty acid esters include, for example, polyoxyethylene stearate, fatty acid polyglycol ester, and the like. These can include polyoxypropylene stearate, polyoxybutylene stearate, polyoxyethylene isostearate, polyoxypropylene isostearate, polyoxyethylene palmitate, and the like.

Illustrative alkanolamides include, for example, lauric acid diethylalkanolamide, palmic acid diethylalkanolamide, and the like. These can include oleic acid diethyalkanolamide, stearic acid diethylalkanolamide, oleic acid diethylalkanolamide, polyethoxylated hydrocarbylamides, polypropoxylated hydrocarbylamides, and the like.

Illustrative polyol fatty acid esters include, for example, glycerol mono-oleate, saturated mono-, di-, and tri-glyceride esters, glycerol mono-stearate, and the like. These can include polyol esters, hydroxyl-containing polyol esters, and the like.

Illustrative borated glycerol fatty acid esters include, for example, borated glycerol mono-oleate, borated saturated mono-, di-, and tri-glyceride esters, borated glycerol monostearate, and the like. In addition to glycerol polyols, these can include trimethylolpropane, pentaerythritol, sorbitan, and the like. These esters can be polyol monocarboxylate esters, polyol dicarboxylate esters, and on occasion polyol tricarboxylate esters. Preferred can be the glycerol mono-oleates, glycerol dioleates, glycerol trioleates, glycerol monostearates, glycerol distearates, and glycerol tristearates and the corresponding glycerol monopalmitates, glycerol dipalmitates, and glycerol tripalmitates, and the respective isostearates, linoleates, and the like. On occasion the glycerol esters can be preferred as well as mixtures containing any of these. Ethoxylated, propoxylated, butoxylated fatty acid esters of polyols, especially using glycerol as underlying polyol can be preferred.

Illustrative fatty alcohol ethers include, for example, stearyl ether, myristyl ether, and the like. Alcohols, including those that have carbon numbers from C<sub>3</sub> to C<sub>50</sub>, can be ethoxylated, propoxylated, or butoxylated to form the cor-

responding fatty alkyl ethers. The underlying alcohol portion can preferably be stearyl, myristyl, C<sub>11</sub>-C<sub>13</sub> hydrocarbon, oleyl, isosteryl, and the like.

The lubricating oils of this disclosure exhibit desired properties, e.g., wear control, in the presence or absence of a friction modifier.

Useful concentrations of friction modifiers may range from 0.01 weight percent to 5 weight percent, or about 0.1 weight percent to about 2.5 weight percent, or about 0.1 weight percent to about 1.5 weight percent, or about 0.1 weight percent to about 1 weight percent. Concentrations of molybdenum-containing materials are often described in terms of Mo metal concentration. Advantageous concentrations of Mo may range from 25 ppm to 700 ppm or more, and often with a preferred range of 50-200 ppm. Friction modifiers of all types may be used alone or in mixtures with the materials of this disclosure. Often mixtures of two or more friction modifiers, or mixtures of friction modifier(s) with alternate surface active material(s), are also desirable.

When lubricating oil compositions contain one or more of the additives discussed above, the additive(s) are blended into the composition in an amount sufficient for it to perform its intended function. Typical amounts of such additives useful in the present disclosure are shown in Table 1 below.

It is noted that many of the additives are shipped from the additive manufacturer as a concentrate, containing one or more additives together, with a certain amount of base oil diluents. Accordingly, the weight amounts in the table below, as well as other amounts mentioned herein, are directed to the amount of active ingredient (that is the non-diluent portion of the ingredient). The weight percent (wt %) indicated below is based on the total weight of the lubricating oil composition.

TABLE 1

| Typical Amounts of Other Lubricating Oil Components |                           |                              |
|-----------------------------------------------------|---------------------------|------------------------------|
| Compound                                            | Approximate wt % (Useful) | Approximate wt % (Preferred) |
| Dispersant                                          | 0.1-20                    | 0.1-8                        |
| Detergent                                           | 0.1-20                    | 0.1-8                        |
| Friction Modifier                                   | 0.01-5                    | 0.01-1.5                     |
| Antioxidant                                         | 0.1-5                     | 0.1-1.5                      |
| Pour Point Depressant (PPD)                         | 0.0-5                     | 0.01-1.5                     |
| Anti-foam Agent                                     | 0.001-3                   | 0.001-0.15                   |
| Viscosity Modifier (solid polymer basis)            | 0.1-2                     | 0.1-1                        |
| Antiwear                                            | 0.2-3                     | 0.5-1                        |
| Inhibitor and Antirust                              | 0.01-5                    | 0.01-1.5                     |

The foregoing additives are all commercially available materials. These additives may be added independently but are usually precombined in packages which can be obtained from suppliers of lubricant oil additives. Additive packages with a variety of ingredients, proportions and characteristics are available and selection of the appropriate package will take the requisite use of the ultimate composition into account.

The following non-limiting examples are provided to illustrate the disclosure.

## EXAMPLES

## Example 1

Formulations were prepared as described herein. All of the ingredients used herein are commercially available. PCMO (passenger car motor oil) formulations were prepared as described herein.

The molybdenum-containing compounds used in the formulations were a low sulfur molybdenum dithiophosphate having a molybdenum to sulfur ratio of 1:1.4 (Molyvan™ L), and a lower sulfur molybdenum dithiophosphate having a molybdenum to sulfur ratio of 1:1.07 (Sakura-Lube™ 300).

The borated ester compound used in the formulations was borated ester (Vanlube™ 289).

The additive package used in the formulations included conventional additives in conventional amounts. Conventional additives used in the formulations were one or more of an antioxidant, dispersant, pour point depressant, detergent, corrosion inhibitor, metal deactivator, seal compatibility additive, anti-foam agent, inhibitor, anti-rust additive, optional friction modifier, optional antiwear additive, and other optional lubricant performances additives.

Formulations were prepared by blending at least one molybdenum-containing compound (e.g., organic molybdenum compound, low sulfur organic molybdenum compound having a molybdenum to sulfur ration of about 1 to less than about 1.1, low sulfur molybdenum dithiophosphate having a molybdenum to sulfur ration of about 1 to less than about 1.1, and optionally a borated ester compound, into a base stock and/or a co-base stock. The additive package was included in several compositions using similar synthetic conditions.

Friction coefficient was measured using a Mini Traction Machine (MTM) manufactured by PCS Instruments. The MTM was operated with a 19.05 mm (3/4 inch) steel ball and a 46 mm diameter steel disc. The slide to roll ratio was fixed at 50% and the speed was varied from 0 to 300 mm/s and repeated for 4 times at 1.0 GPa contact pressure and 140° C. For the 4<sup>th</sup> run, 20 data points were obtained between 0 to 100 mm/s (spaced based on a logarithmic scale). The average of these 20 data points for each formulation was reported in FIGS. 1-4 as the average friction coefficient.

Corrosion protection was determined by a copper strip corrosion test in accordance with ASTM D130. The test was conducted at 150° C. for 3 hours. The test evaluates the degree to which a lubricant will corrode copper-containing materials (e.g., bronze and brass). Results were reported as the comparison to a standard chart in FIGS. 1-4. The standard chart is shown in FIG. 5.

FIG. 1 shows formulations prepared in accordance with the Examples, and the results of MTM testing and copper corrosion testing in accordance with the Examples. In particular, FIG. 1 shows the effects of borated ester (Vanlube™ 289), low sulfur molybdenum dithiophosphate having a molybdenum to sulfur ratio of 1:1.07 (Sakura-Lube™ 300), and low sulfur molybdenum dithiophosphate having a molybdenum to sulfur ratio of 1:1.4 (Molyvan™ L) on copper corrosion and friction coefficients of molybdenum-containing formulations.

Examples 1 and 2 show the effects of borated ester (Vanlube™ 289) on copper corrosion (D130) and friction coefficients. Examples 3-6 show the effects of replacing a low sulfur molybdenum dithiophosphate having a molybdenum to sulfur ratio of 1:1.4 (Molyvan™ L) with a lower sulfur molybdenum dithiophosphate having a molybdenum to sulfur ratio of 1:1.07 (Sakura-Lube™ 300) on copper corrosion (D130) and friction coefficients. Examples 7 and 8 show the synergistic effect of combining low sulfur molybdenum dithiophosphate having a molybdenum to sulfur ratio of 1:1.07 (Sakura-Lube™ 300) and borated ester (Vanlube™ 289) on friction coefficient.

FIG. 2 shows formulations prepared in accordance with the Examples, and the results of MTM testing and copper

corrosion testing in accordance with the Examples. In particular, FIG. 2 shows a comparison of various additives, including corrosion inhibitors, versus borated ester (Vanlube™ 289) on copper corrosion and friction coefficients of molybdenum-containing formulations.

Examples 9 and 10 show the effects of borated ester (Vanlube™ 289) on copper corrosion (D130) and friction coefficients versus other additives (Comparative Examples 4-14).

FIG. 3 shows selected formulations of FIG. 1, and the results of MTM testing and copper corrosion testing of the selected formulations. FIG. 3 shows pictures of copper strips used in the copper corrosion testing in accordance with ASTM D130. FIG. 3 shows that in a lubricant formulation containing 1000 ppm or higher molybdenum, copper corrosion was mitigated by addition of borated ester (Vanlube™ 289) (marketed as an antiwear/antscuff additive and friction reducer) or by use of a low sulfur molybdenum dithiophosphate having a molybdenum to sulfur ratio of 1:1.07 (Sakura-Lube™ 300).

FIG. 4 shows formulations prepared in accordance with the Examples, and the results of MTM testing and copper corrosion testing in accordance with the Examples. In particular, FIG. 4 shows wear metals in used lubricants. The determination of wear metals, contaminants and selected elements in used lubricating oils was conducted in accordance with ASTM D5185.

All patents and patent applications, test procedures (such as ASTM methods, UL methods, and the like), and other documents cited herein are fully incorporated by reference to the extent such disclosure is not inconsistent with this disclosure and for all jurisdictions in which such incorporation is permitted.

When numerical lower limits and numerical upper limits are listed herein, ranges from any lower limit to any upper limit are contemplated. While the illustrative embodiments of the disclosure have been described with particularity, it will be understood that various other modifications will be apparent to and can be readily made by those skilled in the art without departing from the spirit and scope of the disclosure. Accordingly, it is not intended that the scope of the claims appended hereto be limited to the examples and descriptions set forth herein but rather that the claims be construed as encompassing all the features of patentable novelty which reside in the present disclosure, including all features which would be treated as equivalents thereof by those skilled in the art to which the disclosure pertains.

The present disclosure has been described above with reference to numerous embodiments and specific examples. Many variations will suggest themselves to those skilled in this art in light of the above detailed description. All such obvious variations are within the full intended scope of the appended claims.

What is claimed is:

1. A method for improving corrosion protection and friction coefficient in an engine or other mechanical component lubricated with a lubricating oil by using as the lubricating oil a formulated oil, said formulated oil having a composition comprising a lubricating oil base stock comprising a monoester and other synthetic base oil; a viscosity modifier; and a mixture of (i) at least one molybdenum dithiophosphate having a molybdenum to sulfur ratio of about 0.93, and (ii) at least one borated ester, as a minor component; wherein corrosion protection and friction coefficient are improved as compared to corrosion protection and friction coefficient achieved using a lubricating oil containing a minor component other than the mixture of (i) at least

31

one molybdenum dithiophosphate having a molybdenum to sulfur ratio of about 0.93, and (ii) at least one borated ester, wherein the monoester comprises about 20 wt. % of the formulated oil, the combination of the other synthetic base oil and viscosity modifier comprise from about 66.47 to 69.037 wt. % of the formulated oil, the at least one molybdenum dithiophosphate having a molybdenum to sulfur ratio of about 0.93 comprises from 0.763 to 1.526 wt. % of the formulated oil, and the at least one borated ester represented by the following formula:



as well as unreacted glycerol, glycerol mono-, di- and tri-ester,  
unreacted



unreacted boronating agent and unboronated



and comprises from about 0.4 to 1.0 wt. % of the formulated oil, and wherein the formulated oil has a friction coefficient of 0.04 or lower at 140° C., as measured by the Mini Traction Machine (MTM) under a contact pressure of 1.0 GHz, and a copper strip rating of 1A or 1B as measured by ASTM D130 at 150° C.

2. A lubricating oil having a composition comprising a lubricating oil base stock comprising a monoester and other synthetic base oil; a viscosity modifier; and a mixture of (i) at least one molybdenum dithiophosphate having a molybdenum to sulfur ratio of about 0.93, and (ii) at least one borated ester, as a minor component; wherein corrosion

32

protection and friction coefficient are improved as compared to corrosion protection and friction coefficient achieved using a lubricating oil containing a minor component other than the mixture of (i) at least one molybdenum dithiophosphate having a molybdenum to sulfur ratio of about 0.93, and (ii) at least one borated ester,

wherein the monoester comprises about 20 wt. % of the formulated oil, the combination of the other synthetic base oil and viscosity modifier comprise from about 66.47 to 69.037 wt. % of the formulated oil, the at least one molybdenum dithiophosphate having a molybdenum to sulfur ratio of about 0.93 comprises from 0.763 to 1.526 wt. % of the formulated oil, and the at least one borated ester is represented by the following formula:



as well as unreacted glycerol, glycerol mono-, di- and tri-ester,  
unreacted



unreacted boronating agent and unboronated



and comprises from about 0.4 to 1.0 wt. % of the formulated oil, and wherein the formulated oil has a friction coefficient of 0.04 or lower at 140° C., as measured by the Mini Traction Machine (MTM) under a contact pressure of 1.0 GHz, and a copper strip rating of 1A or 1B as measured by ASTM D130 at 150° C.

\* \* \* \* \*